# EUROPEAN PATENT SPECIFICATION

(11) **EP 2 109 008 B1**
(45) Date of publication and mention of the grant of the patent: **14.08.2013**
(21) Application number: 09156818.8
(22) Date of filing: 31.03.2009
(51) Int. Cl.: G03G 9/08, G03G 9/087, G03G 9/09, G03G 9/097, G03G 15/20

(54) **Image formation method**
Bilderzeugungsverfahren
Procédé de formation d'image

(30) Priority: 09.04.2008 JP 2008101110
(43) Date of publication of application: 14.10.2009
(73) Proprietor: Ricoh Company, Ltd., Tokyo 143-8555 (JP)
(72) Inventor: Nakamura, Minoru, Tokyo 143-8555 (JP); Izutani, Akira, Tokyo 143-8555 (JP); Nozaki, Tsuyoshi, Tokyo 143-8555 (JP)
(74) Representative: Barz, Peter

(56) References cited:
- JP-A- 11 002 918
- JP-A- 2002 156 779
- US-A1- 2004 265 718
- US-A1- 2005 053 857

## Description

### BACKGROUND OF THE INVENTION

### Field of the Invention

The present invention relates to an image formation method using a toner.

### Discussion of the Background

In general, methods of fixing a toner image on a recording medium upon application of heat are typified into a contact heat fixing system and a non-contact heat fixing system. The non-contact heat fixing system is a fixing system in which no member contacts with a powder toner image during fixing. Major examples thereof include a flash fixing system and an oven (atmosphere) fixing system. In the flash fixing method, a powder toner image transferred from an image bearing member or an intermediate transfer member to a recording medium is irradiated with flash emitted from a light source, for example, a Xenon or halogen flash lamp, to melt the toner by radiation heat, thereby fixing the powder toner image. In the oven fixing method, a powder toner image transferred from an image bearing member or an intermediate transfer member to a recording medium is irradiated with, for example, infrared in an oven atmosphere, to melt the toner by the radiation heat, thereby fixing the powder toner image on the recording medium.

Such a non-contact heat fixing system has the following advantages.
· Since no member is brought into contact with a powder toner image to melt the toner, image crushing by a member is avoided so that the image definition at development is maintained.
· The fixing time is extremely short, which enables a high speed fixing.
· The waiting time ascribable to fixing can be saved so that the first print (copy) output time can be shortened.
· Dealing with various kind of recording media, for example, having different thickness or paper quality, is easy.

However, the non-contact heat fixing in the non-contact heat fixing system diffuses energy to the outside environment. On the other hand, reducing the fixing energy is an issue in terms of the environment. However, when the total amount of light energy provided to a powder toner image is short, the powder toner image is not sufficiently melted, which leads to deterioration of the fixing property. In addition, controlling the amount of this energy is difficult especially in the case of full color image formation in which a monochrome color image and a full color image are output because the amount of absorption energy varies depending on colors.

In recent years, the particle diameter of toner has been reduced to improve the quality of images. This size reduction of toner particles sacrifices the print density and the fixing property while the amount of toner attached to a recording medium to secure the printing area is reduced. The deterioration of the fixing property, etc. deriving from the size reduction of toner particles is significant in the non-contact heat fixing system in comparison with the contact heat fixing system in which toner is melted by a pressure roller and a heating roller. Furthermore, although the fixing property is desirable for an image such as a solid image having a large amount of attached toner but deteriorates when a toner image such as a character image or a half tone image having a relatively small amount of attached toner is fixed. In addition, this problem is significant for a half tone image in comparison with a character image when the amount of the attached toner is in the same quantity.

When the amount of the energy of a fixing device increases to improve the fixing property, the energy is excessively absorbed at black toner portions, which causes a bumping phenomenon and thus image noise. Additionally, when a recording medium having a fixed image on one side thereof is abraded by a roller, etc. in a paper path, toner bleed and smear, etc. easily occur so that the quality of images deteriorates due to deterioration of anti-smear property.

In addition, non-contact fixing has been demanded recently for color images and gloss images are required in terms of "looking nice" while gloss images are not demanded in the case of monochrome image. This gloss image problem with regard to color images derives from the fixing process in the non-contact fixing because the color particle layer in an image portion is not pressed so that the surface of the image portion is not easily smooth, which leads to deterioration of gloss. In addition, optical absorption efficiency is relatively bad in the case of a color image in comparison with a monochrome image and the colored particle is hardly soluble so that the layer tends not to be smooth, which prevents improvement on gloss. These phenomena are significant when the attached amount of colored particles on an image is small.

There is a typical technology to solve these problems in which a laminate film is attached to the surface of a color image to improve the gloss.

Unexamined published Japanese patent application No. (hereinafter referred to as JOP) H11-2918 describes a technology in which an image having only a small gloss difference between an image portion and a non-image portion is obtained by forming the image on the surface of a recording medium with a colored material containing a coloring agent, etc., transferring an image surface protective material having a thermoplastic resin and a fixing releasing agent to the surface of the recording medium and heating and melting the image surface protective material to form a transparent thin layer and the obtained image is hardly peeled off by abrasion of the image. However, using only an image surface protective material containing a fixing releasing agent, etc., is not sufficient to secure anti-smear property and gloss.

JOP 2002-156779 describes a technology in which an infrared absorption agent is attached to the surface of toner particles for non-contact fixing by heating in an amount of from 0.1 to 1.5 parts by weight based on 100 parts of the toner. The toner is for use in a full color image forming apparatus which fixes the toner on a recording medium by a device for non-contact fixing by heating. Therefore, the toner for non-contact fixing by heating is sufficiently fixed on a recording medium with a reduced amount of the infrared absorption agent, which lowers the manufacturing cost of toner. In addition, the obtained color toner has a uniform charging performance and reduces variation in the color of the color toner and color images having an excellent color reproducibility can be obtained. However, fixating the infrared absorption agent only on the surface of toner particles is not good enough to secure gloss. In Examples, the technology describes that the fixing property of color toner used together with transparent toner is good in the fixing strength test after image formation. However, since the transparent toner has the same characteristics as the color toner with regard to particle diameter, circularity and softening point, the effect of the smoothness is too small to secure gloss.

Therefore, a suitable problem solution has not been provided yet.

### SUMMARY OF THE INVENTION

Because of these reasons, the present inventors recognize that and an image formation method and an image forming apparatus using a non-contact fixing device which have excellent anti-smear property, and deal with a variety of sheets such as thick paper, thin paper, and concavo-convex paper, and no outline images.

Accordingly, an object of the present invention is to provide an image formation method and an image forming apparatus which provides images with good gloss property without vertical streaks or uneven density on a recording medium after fixing and an image formation method and an image forming apparatus using a non-contact fixing device which have excellent anti-smear property, and deal with a variety of sheets such as thick paper, thin paper, and concavo-convex paper, and no outline images.

These and other objects, features and advantages of the present invention will become apparent upon consideration of the following description of the preferred embodiments of the present invention taken in conjunction with the accompanying drawings.

### BRIEF DESCRIPTION OF THE DRAWINGS

Various other objects, features and attendant advantages of the present invention will be more fully appreciated as the same becomes better understood from the detailed description when considered in connection with the accompanying drawings in which like reference characters designate like corresponding parts throughout and wherein:
Fig. 1 is a schematic diagram illustrating an example of an image forming apparatus;
Fig. 2 is a schematic diagram illustrating an example of the development device for use in the present invention;
Fig. 3 is a schematic diagram illustrating an example of the non-contact fixing device for use in the present invention; and
Fig. 4 is a schematic diagram illustrating an example of the process cartridge for use in the present invention.

### DETAILED DESCRIPTION OF THE INVENTION

The present invention will be described below in detail with reference to several embodiments and accompanying drawings.

The image formation method of the present invention has: a process of developing a latent image on an image bearing member with a toner containing a coloring agent, a first binder resin, ; a process of transferring the toner to a recording medium; a process of transferring a fixing helping particle including a second binder resin, to the recording medium after transferring the toner to the recording medium; and a process of fixing the toner and the fixing helping particle on the recording medium. In addition, the toner and the fixing helping particle satisfy the following relationships: $6 μm \geq Dvc \geq 3 μm$ $Dvc > 10 \times Dvt$ $Sc < St ,$ $6 μm \geq Dvc \geq 3 μm$ $Dvc > 10 \times Dvt$ $Sc < St ,$ wherein Dvc represents the volume average particle diameter of the toner, Dvt represents the volume average particle diameter of the fixing helping particle, Sc represents the average circularity of the toner and St represents the average circularity of the fixing helping particle.

The toner has a volume particle diameter of from 3 to 6 µm and preferably from 4 to 6 µm. A volume particle diameter that is too small may have an adverse impact on each process of the image formation process. A volume particle diameter that is too large may degrade the definition of an image.

The fixing helping particle has a volume particle diameter less than one tenth of the volume particle diameter of the toner and preferably from less than one fifteenth to greater than fiftieth thereof. When the volume particle diameter of the fixing helping particle is too large, the fixing helping particle hardly sets in the concave portion of a convexo-concave portion of a color image so that the color image does not form a smooth surface, which causes uneven gloss.

In addition, the fixing helping particle for use in the present invention has an average circularity greater than that of the toner, meaning that the fixing helping particle is closer to a sphere than the toner. When the fixing helping particle has an average circularity less than the toner, meaning more irregular form, the fluidity of the fixing helping particle deteriorates and therefore the fixing helping agent does not easily set in the concave portion of a convexo-concave portion of a color image so that the color image does not form a smooth surface, which causes uneven gloss. Furthermore, the fixing helping particle tends to be difficult to densely contact with the toner and thus, the fixing helping particle does not easily receive the thermal energy of the toner. Therefore, the image is not fixed with a small amount of energy and thus does not form a smooth surface. That is, securing gloss of a color image with a small amount of energy is difficult.

In addition, in the image formation method using a non-contact fixing device (mechanism), when the attachment amount of the toner forming an image on a recording medium is small, the image formed of the toner tends to have a rough surface (a large difference between the top and the bottom of the convexo-concave portion) so that the image does not form a smooth surface, causing a problem of poor gloss.

In addition, the image formation method using a non-contact fixing device (mechanism) of the present invention includes: a process of transferring a toner containing a first binder resin, a coloring agent, a first infrared absorption agent, to a recording medium; thereafter transferring a fixing helping particle containing a second binder resin, a second infrared absorption agent, to the recording medium; and a process of fixing in a non-contact manner. In addition the toner and the fixing helping particle satisfies the relationships described above and therefore, the image formation method provides good gloss and good anti-smear property.

In the present invention, the toner and the fixing helping particle effectively absorb optical energy and converts it into thermal energy which is enough to melt toner particles one by one.

When the amount of toner attached is relatively small (for example, when an image having a portion having a low density is formed or the entire amount of toner attached to a solid portion is reduced), for example, 2 g/m² or less, a problem arises that the fixing property deteriorates. This phenomenon is considered to occur because toner particles are isolated on a recording medium and part of radiation heat escapes to the recording medium or outside so that a sufficient amount of the radiation heat is not secured to melt the toner while when toner particles are densely present on a recording medium, for example, around 5 g/m² or less, the heat hardly escapes to the surrounding and is conveyed from toner particles to toner particles, which secures sufficient fixing.

However, in the present invention, toner is sufficientlymelted one particle by one particle as described above, the toner penetrates into a recording medium even when the amount of toner attached to the recording medium is reduced or toner particles are isolated from each other on the recording medium. Therefore, the toner is efficiently fixed on a recording medium as a full color toner for non-contact heat fixing. The fixing helping particle for use in the present invention has a volume particle diameter less than one tenth of the volume particle diameter of the toner and is closer to a sphere than the toner. Therefore, the fixing helping agent easily sets in the concave portion of a convexo-concave portion of a color image formed of the toner. Furthermore, the fixing helping particle tends to densely contact with the toner and thus, the fixing helping particle easily receives the thermal energy of the toner. Therefore, the image is fixed with a small amount of thermal energy and thus forms a smooth surface. Since the fixing helping particle is significantly transparent, the image looks an image formed of only the toner. The fixing helping particles are present around the toner, which helps preventing the heat from escaping into the surrounding. Therefore, anti-smear property is secured even when the attachment amount of the fixing helping agent is small. In addition, the fixing helping agent is easily melted so that the degree of smoothness is improved and sufficient gloss is secured. A fine fixed full color image with good anti-smear property and gloss is obtained with a relatively small fixing energy of, for example, from 3 to 5 J/cm².

The fixing helping particle preferably has a particle diameter distribution with a ratio of the volume average particle diameter to the number average particle diameter greater than 1.4. That is, the fixing helping particle has a wide particle diameter distribution. Having such a particle diameter distribution, the fixing helping particle is densely filled so that a small particle easily fits in the gap between large particles. In addition, particles densely contact with each other and thus the toner and the fixing helping particles can be melted with a small amount of energy, which improves gloss and anti-smear property of a toner.

The toner for use in the present invention includes a binder resin, a coloring agent, and an infrared absorption agent is preferably contained in the case of the image formation method using a non-contact fixing device. The infrared absorption agent for use in the toner for use in the present invention represents an agent having an absorption peak in the wavelength range of from 700 to 1,100 nm. The infrared absorption agent is selected to have an absorption wavelength in the oscillation wavelength of a light source.

Specifically, the infrared absorption agent is selected from the group consisting of a cyanine based compound, a polymethine based compound, an aminium based compound, a diimonium based compound, a phthalocyanine based compound, a merocyanine based compound, a benzenethiol based metal complex, a mercaptophenol based metal complex, an aromatic diamine based metal complex, a nickel complex compound, an anthraquinone based compound, a naphthalocyanine based compound, and an indolenine compound.

In the present invention, among the compounds specified above, using a compound having an absorption peak in the wavelength range of from 800 to 1,000 nm is preferred in terms of efficient optical absorption. More preferably, the toner of the present invention contains at least two compounds having respective maximum absorption wavelengths as the infrared absorption agent. To be specific, it is more preferred to use at least a compound having an absorption peak in the wavelength range of from 800 to 870 nm and more preferably from 810 to 840 nm in a particularly preferred combination with a compound having an absorption peak in the wavelength range of from 870 to 1, 000 nm and more preferably from 900 to 980 nm.

Specific examples of the compounds having an absorption peak in the wavelength range of from 800 to 870 nm include, but are not limited to, a polymethine based compound (R-820B, manufactured by NipponKayakuCo., Ltd.), cyanine based compounds (CY-2, CY-4 and CV-9, manufactured by Nippon Kayaku Co., Ltd.), and an indolenine compound.

The indolenine compound is preferred in terms that optical energy is effectively absorbed even when the amount of the optical energy is small and the side effect on the color reproducibility for a color toner is small. Since the indolenine compound has a sharp peak in the absorption spectrum thereof, the light in a desired wavelength range can be efficiently absorbed and also the indolenine compound is preferred because the absorption thereby is little in the optical part of the spectrum.

Specific examples of the compounds having an absorption peak in the wavelength range of from 870 to 1,000 nm include, but are not limited to, a diimonium based compound (NIR-AM1 and NIR-IM1 manufactured by Nagase Chemtex Corporation, IRG-022 and IRG-023, manufactured by Nippon Kayaku Co., Ltd.), phthalocyanine based compounds (TX-305A, manufactured by Nippon Shokubai Co., Ltd.), and an aminium based compound (CIR-960 and CIR-961, manufactured by Japan Carlit Co., Ltd., IRG-002, IRG-003 and IRG-003K, manufactured by preferred in terms that optical energy is effectively absorbed even when the amount of the optical energy is small and the side effect on the color reproducibility for a color toner is less.

The total addition amount of the infrared absorption agent is from 0.01 to 2 parts by weight and preferably from 0.1 to 1 part by weight to obtain a good fixing property without having an adverse impact on the color reproducibility, the charging property, the cost, . In addition, the ratio of the two kinds of the infrared absorption agents (the addition amount of the infrared absorption agent having the maximum absorbency in the wavelength range of from 800 to 870 nm to the addition amount of the infrared absorption agent having the maximum absorbency in the wavelength range of from 870 to 1,000 nm) is from 1 : 4 to 4 : 1 and preferably from 1 : 3 to 2 : 1 to improve the fixing property by a small amount of the infrared absorption agents.

The toner for use in the present invention preferably has an average circularity of 0.95 or higher. An average circularity that is too small may lead to a bad transfer.

The toner for use in the present invention contains a binder resin, a coloring agent, an infrared absorption agent, and an external additive is added to the toner. External additives improve fluidity, developabililty and transferability.

The product of the volume average particle diameter of the toner and the addition amount of such an external additive is preferably from 3 to 18 µm % by weight. An excessively small product tends to

The product of the volume average particle diameter of the toner and the addition amount of such an external additive is preferably from 3 to 18 µm ·% by weight. An excessively small product tends to degrade the transferability, which leads to production of images having hollow defects. This hollow defect easily occurs especially when a full color image is formed or a toner containing a releasing agent is used. When this product is too large, the fixing property tends to degrade and the fixing strength of a produced image is easily insufficient. The fixing strength easily deteriorates especially when a half tone image having a small attachment amount is fixed by a non-contact fixing device.

In addition, the toner of the present invention is suitable for dealing with various kinds of media from thin media to thick media to rough media and brimless images.

In the present invention, the transferability represents the degree of easiness of transfer when a toner image formed on the surface of an image bearing member is transferred to a transfer body. In addition, when a toner image on the surface of an image bearing member is once transferred to an intermediate transfer body such as an intermediate transfer belt and thereafter the toner image on the intermediate transfer body is transferred to a recording medium, the transferability represents the degree of easiness of transfer from the image bearing member to the intermediate transfer body and from the intermediate transfer mediate body to the recording medium.

The toner for use in the present invention preferably employs a core shell stricture. Such a core shell structure is formed of, for example, a core containing a coloring agent, an infrared absorption agent and a binder resin (A) and a shell having a binder resin (B) which covers the core. It is preferable that the binder resin (A) is mainly made of a polyester based resin and the binder resin (B) is a vinyl based copolymer. That is, the core forming the main component of toner includes a polyester based resin because the polyester based resin is advantageous in terms of a combination of the low temperature fixing property and the high temperature preservability and the shell portion, which has a significant impact on the chargeability of toner, includes a vinyl based copolymer since the vinyl based copolymer is preferred to control the chargeability.

Due to such a core shell structure, the infrared absorption agent present and the infrared absorption agent do not expose to the surface of the toner. Furthermore, when a latent electrostatic image is developed by using a development roller having a relatively small diameter in a single component development system, the shell portion absorbs the pressure applied to the toner, thereby preventing toner cracking and transformation.

### Polyester resin

There is no specific limit to the kind of the polyester resin for use in the present invention and any kinds of polyester resins can be used. Also, a mixture of several kinds of polyester resins can be used. Specific examples of the polyester resins include, but are not limited to, condensation products of the following polyols (1) and the polycarboxylic acids (2).

### Polyol

Specific examples of the polyols (1) include, but are not limited to, alkylene glycol (e.g., ethylene glycol, 1,2-propylene glycol, 1,3-propylene glycol, 1,4-butanediol and 1,6-hexanediol); alkylene ether glycols (e.g., diethylene glycol, triethylene glycol, dipropylene glycol, polyethylene glycol, polypropylene glycol and polytetramethylene ether glycol); alicyclic diols (e.g., 1, 4-cyclohexane dimethanol and hydrogenated bisphenol A) ; bisphenols (e.g., bisphenol A, bisphenol F, and bisphenol S), 4,4^{'} -dihydroxybiphenyls such as 3,3-difluoro-4,4^{'} -dihydroxybiphenyl; bis(hydroxyphenyl)alkanes such as bis(3-fluoro-4-hydroxyphenyl)methane, 1-phenyl-1,1^{'} -bis(3-fluoro-4-hydroxyphenyl)ethane, 2,2-bis(3-fluoro-4-hydroxyphenyl)propane, 2,2-bis(3,5-difluoro-4-hydroxyphenyl)propane (also referred to as tetrafluorobisphenol A), and 2,2-bis(3-hydroxyphnyl)-1,1,1,3,3,3-hexafluoropropane; bis(4-hydorxyphenyl)ethers such as bis(3-fluoro-4-hydroxyphenyl)ether; adducts of the alicyclic diols mentioned above with an alkylene oxide (e.g., ethylene oxide, propylene oxide and butylene oxide); and adducts of the bisphenols mentioned above with an alkylene oxide (e.g., ethylene oxide, propylene oxide and butylene oxide); .

Among these compounds, alkylene glycols having from 2 to 12 carbon atoms and adducts of a bisphenol with an alkylene oxide are preferable. More preferably, adducts of a bisphenol with an alkylene oxide, or mixtures of an adduct of a bisphenol with an alkylene oxide and an alkylene glycol having from 2 to 12 carbon atoms can be used.

Specific examples of the aliphatic polyols having three or more hydroxyl groups include, but are not limtied to, glycerin, trimethylol ethane, trimethylol propane, pentaerythritol and sorbitol); polyphenols having three or more hydroxyl groups (trisphenol PA, phenol novolak and cresol novolak); and adducts of the polyphenols having three or more hydroxyl groups mentioned above with an alkylene oxide.

The polyols specified above can be used alone or in combination.

### Polycarboxylic Acids

Specific examples of the polycarboxylic acids (2) include, but are not limited to, alkylene dicarboxylic acids (e.g., succinic acid, adipic acid and sebacic acid); alkenylene dicarboxylic acids (e.g., maleic acid and fumaric acid) ; and aromatic dicarboxylic acids (e.g., phthalic acid, isophthalic acid, terephthalic acid, naphthalene dicarboxylic acids, 3-fluoroisophtahlic acid, 2-fluoroisophthalic acid, 2-fluoroterephtahlic acid, 2,4,5,6-tetrafluoroisophtahlic acid, 2,3,5,6-tetrafluoro terephthalic acid, 5-trifluoromthyl isophthalic acid, 2,2-bis(4-carboxyphenyl)hexafluoropropane, 2,2-bis(4-carboxyphenyl)hexafluoro propane, 2,2-bis(3-carboxyphenyl)hexafluoropropane, 2,2^{'} -bis(trifluoromethyl)-4,4^{'} -biphenyl dicarboxylic acid, 3,3^{'} -bis(trifluoromethyl)4,4^{'} -biphenyl dicarboxylic acid, 2,2^{'} -bis(trifluoromethyl)-3,3^{'} -biphenyl dicarboxylic acid, and hexafluoro isopropylidene diphthalic anhydride).

Among these compounds, alkenylene dicarboxylic acids having 4 to 20 carbon atoms and aromatic dicarboxylic acids having 8 to 20 carbon atoms are preferably used. Specific examples of the polycarboxylic acids having three or more hydroxyl groups include, but are not limited to, aromatic polycarboxylic acids having 9 to 20 carbon atoms (e.g., trimellitic acid and pyromellitic acid).

Anhydrides or lower alkyl esters (e.g., methyl esters, ethyl esters or isopropyl esters) of the polycarboxylic acids specified above can be used for the reaction with a polyol (1) to obtain the polycarboxylic acid.

The polycarboxylic acids specified above can be used alone or in combination and are not limited to the specified above.

### Ratio of Polyol and Polycarboxylic Acid

The suitable mixing ratio (i.e., an equivalence ratio [OH]/[COOH]) of a polyol (PO) to a polycarboxylic acid (PC) is from 2/1 to 1/1, preferably from 1.5/1 to 1/1 and more preferably from 1.3/1 to 1.02/1.

### Molecular weight of Polyester Resin

The peak molecular weight is from 1,000 to 30, 000, preferably from 1,500 to 10,000 and more preferably from 2,000 to 8,000. When the peak molecular weight is too small, the high temperature of the toner tends to deteriorate. When the peak molecular weight is too large, the low temperature fixing property easily deteriorates.

### Vinyl Based Copolymer Resin

There is no specific limit to the selection of the vinyl based copolymer resins for use in the present invention and any can be used. Also, a mixture of several kinds of vinyl based copolymer resins can be used.

The vinyl based copolymer resins are copolymerized polymers of vinyl based monomers. Specific examples of the vinyl based monomers include, but are not limited to, the following (1) to (10).

### (1) Vinyl Based Hydrocarbon

Aliphatic vinyl based hydrocarbons: alkenes such as ethylene, propylene, butane, isobutylene, pentene, heptene, diisobutylene, octane, dodecene, octadecene, α-olefins other than the above mentioned; alkadiens such as butadiene, isoplene, 1,4-pentadiene, 1,6-hexadiene, and 1,7-octadiene

Alicyclic vinyl based hydrocarbons: mono- or di- cycloalkenes and alkadiens such as cyclohexene, (di)cyclopentadiene, vinylcyclohexene, and ethylidene bicycloheptene; and terpenes such as pinene, limonene and indene.

Aromatic vinyl-based hydrocarbons: styrene and its hydrocarbyl (alkyl, cycloalkyl, aralkyl and/or alkenyl) substitutes, such as α -methylstyrene, vinyl toluene, 2,4-dimethylstyrene, ethylstyrene, isopropyl styrene, butyl styrene, phenyl styrene, cyclohexyl styrene, benzyl styrene, crotyl benzene, divinyl benzene, divinyl toluene, divinyl xylene, and trivinyl benzene; and vinyl naphthalene.

### (2) Vinyl Based Monomer Containing Carboxyl Group and its Salts

Unsaturated mono carboxylic acid and unsaturated dicarboxylic acid having 3 to 30 carbon atoms, and their anhydrides and their monoalkyl (having 1 to 24 carbon atoms) esters, such as vinyl based monomers having carboxylic group such as (meth)acrylic acid, (anhydride of) maleic acid, mono alkyl esters of maleic acid, fumaric acid, mono alkyl esters of fumaric acid, crotonic acid, itaconic acid, mono alkyl esters of itaconic acid, glycol monoether of itaconic acid, mono alkyl esters of citraconic acid and bvinyl based monomer containing carboxyl group of cinnamic acid, .

### (3) Vinyl Based Monomer Having Sulfonic Group, Monoesterified Vinyl Based Sulfuric Acid and their Salts

Alkene sulfuric acid having 2 to 14 carbon atoms such as vinyl sulfuric acid, (meth) aryl sulfuric acid, methylvinylsufuric acid and styrene sulfuric acid; their alkyl derivatives having 2 to 24 carbon atoms such as α-methylstyrene sulfuric acid; sulfo(hydroxyl)alkyl-(meth)acrylate or (meth)acryl amide such as sulfopropyl(meth)acrylate, 2-hydroxy-3-(meth)acryloxy propylsulfuric acid, 2-(meth)acryloylamino-2,2-dimethylethane sulfuric acid, 2-(meth)acryloyloxyethane sulfuric acid, 3-(meth)acryloyloxy-2-hydroxypropane sulfuric acid, 2-(meth)acrylamide-2-methylpropane sulfuric acid, 3-(meth)avrylamide-2-hydroxy propane sulfuric acid, alkyl (having 3 to 18 carbon atoms) aryl sulfosuccinic acid, sulfuric esters of poly (n = 2 to 30) oxyalkylene (ethylene, propylene, butylenes: (mono, random, block) mono(meth)acrylate such as sulfuric acid ester of poly (n = 5 to 15) oxypropylene monomethacrylate, and sulfuric acid ester of polyoxyethylene polycyclic phenyl ether.

### (4) Vinyl Based Monomer Having Phosphoric Group and its Salts

Phosphoric acid monoester of (meth)acryloyl oxyalkyl such as 2-hydroxyethyl(meth)acryloyl phosphate, phenyl-2-acyloyloxyethylphosphate, (meth) acryloyloxyalkyl (having 1 to 24 carbon atoms) phosphonic acids such as 2-acryloyloxy ethylphosphonic acid and their salts, .

Specific examples of the salts of the compounds of (2) to (4) include, but are not limited to, alkali metal salts (sodium salts, potassium salts, ), alkali earth metal salts (calcium salts, magnesium salts), ammonium salts, amine salts, quaternary ammonium salts, .

### (5) Vinyl Based Monomer Having Hydroxyl Group

Hydroxystyrene, N-methylol(meth)acryl amide, hydroxyethyl(meth)acrylate, (meth)arylalcohol, crotyl alcohol, isocrotyl alcohol, 1-butene-3-ol, 2-butene-1-ol, 2-butene-1,4-diol, propargyl alcohol, 2-hydroxyethylpropenyl ether, simple sugar aryl ether, .

### (6) Vinyl Based Monomer Having Nitrogen

Vinyl based monomer having an amino group: aminoethyl(meth)acrylate, dimethylaminoethyl(meth)acrylate, diethylaminoethyl(meth)acrylate, t-butylaminoethyl(meth)acrylate, N-aminoethyl(meth)acrylamide, (metha)arylamine, morpholino ethyl (meth) acrylate, 4-vinylpyridine, 2-vinylpyridine, crotyl amine, N,N-dimethylaminostyrene, methyl-α-acetoaminoacrylate, vinylimidazole, N-vinylpyrrole, N-vinylthiopyrolidone, N-arylphenylene diamine, aminocarbozole, aminothiazole, aminoindole, aminopyrrole, aminoimidazole, and aminomercaptothiazole and their salts.

Vinyl Based Monomer Having Amide Group: (meth)acrylamide, N-methyl(meth)acrylamide, N-butylacrylamide, diacetone acrylamide, N-methylol(meth)acrylamide, N,N-methylene-bis(meth)acrylamide, cinnamic amide, N,N-dimethylacrylamide, N,N-dibenzylacrylamide, methacrylformamide, N-methyl-N-vinylacetoamide, and N-vinylpyrolidone.

Vinyl Based Monomer Having Nitrile Group: (meth) acrylonitrile, cyanostyrene and cyanoacrylate.

Vinyl Based Monomer Having Quaternary Ammonium Group: quaternarized vinyl based monomer having tertiary amine group such as dimethylaminoethyl(meth)acrylate, diethylaminoethyl(meth)acrylate, dimethylaminoethyl(meth)acrylamide, diethylaminoethyl(meth)acrylamide, diarylamine, (quaternaized by using a quaternarizing agent such as methylchloride, dimethyl sulfuric acid, benzyl chloride, dimethylcarbonate).

Vinyl Based Monomer Having Nitro Group: nitrostyrene,

### (7) Vinyl Based Monomer Having Epoxy Group

Glycidyl (meth)acrylate, tetrahydrofurfuryl(meth)acrylate, and p-vinylphenyl phenyloxide.

### (8) Vinyl Esters, Vinyl(thio)ether, Vinylketone, Vinyl Sulfonic Acid

Vinyl esters: Vinyl acetate, vinyl butylate, vinyl propionate, vinyl butyrate, diarylphthalate, diaryladipate, isopropenyl acetate, vinylmethacrylate, methyl-4-vinylbenzoate, cyclohexylmethacrylate, benzylmethacrylate, phenyl(meth)acrylate, vinylmethoxyacetate, vinylbenzoate, ethyl-α-ethoxyacrylate, alkyl (having 1 to 50 carbon atoms) (meth)acrylate such as methyl(meth)acrylate, ethyl(meth)acrylate, propyl(meth)acrylate, butyl(meth)acrylate, 2-ethylhexyl(meth)acrylate, dodecyl(meth)acrylate, hexadecyl(meth)acrylate, heptadecyl(meth)acrylate, and eicocyl (meth) acrylate), dialkyl malate (in which two alkyl groups are straight chained, branch chained, or cyclic chained groups and have 2 to 8 carbon atoms), poly(meth)aryloxyalkanes such as diaryloxyethane, triaryloxyethane, tetraaryloxyethane, tetraaryloxypropane, tetraaryloxybutane and tetrametharyloxyethane, vinyl based monomers having polyalkylene glycol chain such as polyethylene glycol (molecular weight: 300) mono(meth)acrylate, polypropylene glycol (molecular weight: 500) monoacrylate, adducts of (meth)acrylate with 10 mol of methylalcoholethyleneoxide, and adducts of (meth)acrylate with 30 mol of lauryl alcohol ethylene oxide), poly(meth)acrylates such as poly (meth) acrylates of polyhydroxyl alcohols (e.g., ethylene glycol di(meth)acrylate, propylene glycol di(meth)acrylate, neopentylglycol di(meth)acrylate, trimethylol propane tri(meth)acrylate, and polyethylene glycol di(meth)acrylate).

Vinyl(thio)ethers: vinylmethyl ether, vinylethyl ether, vinylpropyl ether, vinylbutyl ether, vinyl-2-ethylhexyl ether, vinylphneyl ether, vinyl-2-methoxyethyl ether, methoxy butadiene, vinyl-2-buthxyethyl ether, 3,4-dihydro-1,2-pyrane, 2-buthoxy-2^{'} -vinyloxy diethyl ether, vinyl-2-ethylmercapto ethylether, acetoxystyrene and phenoxy styrene.

Vinyl ketones: vinyl methylketone, vinylethylketone, and vinyl phenylketone.

Vinyl sulfone: divinyl sulfide, p-vinyl diphenyl sulfide, vinyl ethylsulfide, vinyl ethylsulfone, divinyl sulfone, and divinyl sulfoxide.

### (9) Other Vinyl Based Monomer

Isocyanate ethyl(meth)acrylat, and m-isopropenyl-α,α -dimethylbenzyl isocyanate.

### (10) Vinyl Based Monomer Having Fluorine Atom

4-fluorostyrene, 2,3,5,6-tetrafluorostyrene, pentafluorophenyl(meth)acrylate, pentafluorobenzyl(meth)acrylate, perfluorocyclohexyl(meth)acrylate, perfluorocyclohexylmethyl(meth)acrylate, 2,2,2-trifluoroethyl(meth)acrylate, 2,2,3,3-tetrafluoropropyl(meth)acrylate, 1H,1H,4H-hexafluorobutyl(meth)acrylate, 1H,1H,4H-hexafluorobutyl(meth)acrylate, 1H,1H,5H-ocatafluoropentyl(meth)acrylate, 1H,1H,7H-dodecafluoroheptyl(meth)acrylate, perflurooctyl(meth)acrylate, 2-perfluorooctylethyl(meth)acrylate, heptadecafluorodecyl(meth)acrylate, trihydroperfluoroundecyl(meth)acrylate, perfluoronorbonyl(meth)acrylate, 1H-perfluoroisobornyl(meth)acrylate, 2-(N-butylperfluorooctane sulfone amide)ethyl(meth)acrylate, 2-(N-ethylperfluorooctane sulfone amide)ethyl(meth)acrylate, and derivatives introduced from α-fluoroacrylic acid.

Bis-hexafluoroiso propyl itaconate, bis-hexafluoro isopropyl malate, bis-perfluorooctyl itaconate, bis-perfluorooctyl malate, bis-trifluoroethyl itaconate, and bis-trifluoroethyl malate.

Vinylheptafluorobutylate, vinyl perfluoroheptanoate, vinyl perfluoro nonanoate and vinyl perfluoro octanoate.

### Vinyl Based Copolymer

As copolymers of a vinyl based monomer, copolymerized polymers formed of any two or more monomers of the compounds of (1) to (10) with an arbitral ratio can be used. Specific examples thereof include, but are not limited to, ester copolymers of styrene and (meth) acrylic acid, styrene-butadiene copolymers, ester copolymers of (meth)acrylic acid and acrylic acid, copolymers of styrene and acrylonitrile, copolymers of styrene and anhydride of maleic acid, copolymers of styrene and (meth)acrylic acid, copolymers of styrene and (meth)acrylic acid and divinyl benzene, and ester copolymers of styrene, styrene sulfonic acid and (meth)acrylic acid. Vinyl Based Copolymer Resin Particulate

It is preferable to use vinyl based copolymer resin particulates dispersed in an aqueous medium as the vinyl based copolymers specified above for use in manufacturing the toner. Vinyl based copolymer resin particulates are easily manufactured by a typical emulsification polymerization. In addition, the binder resin (B) in the toner of the present invention is preferably formed by agglomeration and/or adhesion of particulates formed of a vinyl based copolymer resin. The core portion can be tightly, smoothly and evenly covered by using the agglomeration body of particulates as the shell portion and more tightly, smoothly and evenly covered when an adhesion body of particulates is used instead. This has a good impact on stability of the charge amount distribution and improvement on transferability.

### Modified Polyester Resin

The binder resin (A) specified above for use in the present invention may include a polyester resin elongated by urethane and/or urea linkage (hereinafter referred to as a modified polyester resin having an urethane and/or urea group) to adjust the viscosity and elasticity for prevention of offset. The content ratio of the modified polyester resin having an urethane and/or urea group in the binder resin (A) specified above is preferably not greater than 20 % by weight. A content ratio that is too high tends to degrade the low temperature fixing property. A content ratio that is too low easily leads to deterioration of compression strength. The modified polyester resin having an urethane and/or urea group can be directly mixed with the binder resin (A) but is preferably manufactured by mixing a modified polyester having an isocyanate group at its end and a relatively low molecular weight (hereafter referred to as prepolymer), an amine reactive therewith and the binder resin (A) followed by elongation reaction and/or cross-linking reaction during or after granulation to obtain a modified polyester resin having an urethane and/or urea group. Thereby, a modified polyester resin having a relatively high molecular weight for use in adjustment of viscosity and elasticity can be easily contained in the core portion. Prepolymer

The polyester prepolymer mentioned above can be prepared by, for example, reacting a polyester having an active hydrogen group, which is a polycondensation product of a polyol (1) and a polycarboxylic acid (2), and a polyisocyanate (3). Specific examples of the active hydrogen group contained in the polyester mentioned above including the mentioned above include, but are not limited to, hydroxyl groups (alcohol hydroxyl groups and phenol hydroxyl groups), amino groups, carboxylic groups, and mercarpto groups. Among these, alcohol hydroxyl groups are particularly preferred.

### Polyisocyanate

Specific examples of the polyisocyanates (3) include, but are not limited to, aliphatic polyisocyanates (e.g., tetramethylene diisocyanate, hexamethylene diisocyanate and 2,6-diisocyanate methylcaproate); alicyclic polyisocyanates (e.g., isophorone diisocyanate and cyclohexylmethane diisocyanate); aromatic diisosycantes (e.g., tolylene diisocyanate and diphenylmethane diisocyanate); aromatic aliphatic diisocyanates (e.g., α,α,α^{'}, α ^{'} -tetramethyl xylylene diisocyanate); isocyanurates; blocked polyisocyanates in which the polyisocyanates mentioned above are blocked with phenol derivatives thereof, oximes or caprolactams; These compounds can be used alone or in combination.

### Ratio of Isocyanate Group and Hydroxyl Group

Suitable mixing ratio (i.e., [NCO]/[OH]) of a polyisocyanate (PIC) to a polyester having a hydroxyl group is from 5/1 to 1/1, preferably from 4/1 to 1.2/1 and more preferably from 2.5/1 to 1.5/1. When the [NCO] / [OH] ratio is too large, the low temperature fixability of the toner tends to deteriorate. When the molar ratio of [NCO] is too small, the urea content of a modified polyester tends to be small and the hot offset resistance easily deteriorates.

The content of the constitutional component of a polyisocyanate (PIC) in the polyester prepolymer (A) having a polyisocyanate group at its end portion is from 0.5 to 40 % by weight, preferably from 1 to 30 % by weight and more preferably from 2 to 20 % by weight. When the content is too low, the hot offset resistance of the toner easily deteriorates. In contrast, when the content is too high, the low temperature fixability of the toner tends to deteriorate. Number of Isocyanate Groups in Prepolymer

The number of isocyanate groups included in the prepolymer (A) per molecule is normally not less than 1, preferably from 1.5 to 3, and more preferably from 1.8 to 2.5. When the number of isocyanate groups is too small, the molecular weight of urea-modified polyester tends to be small and the hot offset resistance easily deteriorates. Elongation Agent and/or Cross Linking Agent

In the present invention, amines can be used as an elongation agent and/or a cross linking agent. Specific examples of the amines (B) include, but are not limited to, diamines (B1), polyamines (B2) having three or more amino groups, amino alcohols (B3), amino mercaptans (B4), amino acids (B5), and blocked amines (B6) in which the amines (B1-B5) mentioned above are blocked.

Specific examples of the diamines (B1) include, but are not limited to, aromatic diamines (e.g., phenylene diamine, diethyltoluene diamine, 4,4^{'} -diaminodiphenyl methane, tetrafluoro-p-xylylene diamine, and tetrafluoro-p-phenylene diamine); alicyclic diamines (e.g., 4,4^{'} -diamino-3,3^{'} -dimethyldicyclohexyl methane, diaminocyclohexane and isophoron diamine); aliphatic diamines (e.g., ethylene diamine, tetramethylene diamine, hexamethylene diamine, dodecafluorohexylene diamine, and tetracosafluorododecylene diamine);

Specific examples of the polyamines (B2) having three or more amino groups include, but are not limited to, diethylene triamine, and triethylene tetramine.

Specific examples of the amino alcohols (B3) include, but are not limited to, ethanol amine and hydroxyethyl aniline.

Specific examples of the amino mercaptan (B4) include, but are not limited to, aminoethyl mercaptan and aminopropyl mercaptan.

Specific examples of the amino acids (B5) include, but are not limited to, amino propionic acid and amino caproic acid.

Specific examples of the blocked amines (B6) include, but are not limited to, ketimine compounds which are prepared by reacting one of the amines B1-B5 mentioned above with a ketone such as acetone, methyl ethyl ketone and methyl isobutyl ketone; oxazoline compounds.

### Molecular Weight Control Agent

Furthermore, the molecular weight of the modified polyesters after the cross linking reaction and/or the elongation reaction can be controlled by using a molecular-weight control agent, if desired. Specific examples of the molecular-weight control agent include, but are not limited to, monoamines (e.g., diethyl amine, dibutyl amine, butyl amine and lauryl amine), and blocked amines (i.e., ketimine compounds) prepared by blocking the monoamines mentioned above.

### Ratio of Amino Group and Isocyanate Group

The mixing ratio of the isocyanate group to the amines (B), i.e., the equivalent ratio ([NCO]/[NHx]) of the isocyanate group [NCO] contained in the prepolymer (A) to the amino group [NHx] contained in the amines (B), is normally from 1/2 to 2/1, preferably from 1.5/1 to 1/1.5 and more preferably from 1.2/1 to 1/1.2. When the mixing ratio is too large or too small, the molecular weight of the resultant urea-modified polyester (i) decreases, resulting in deterioration of the hot offset resistance of the resultant toner.

### Coloring Agent

Suitable coloring agents (coloring material) for use in the toner of the present invention include known dyes and pigments. Specific examples of the coloring agents include, but are not limited to, carbon black, Nigrosine dyes, black iron oxide, Naphthol Yellow S, Hansa Yellow (10G, 5G and G), Cadmium Yellow, yellow iron oxide, loess, chrome yellow, Titan Yellow, polyazo yellow, Oil Yellow, Hansa Yellow (GR, A, RN and R), Pigment Yellow L, Benzidine Yellow (G and GR), Permanent Yellow (NCG), Vulcan Fast Yellow (5G and R), Tartrazine Lake, Quinoline Yellow Lake, Anthrazane Yellow BGL, isoindolinone yellow, red iron oxide, red lead, orange lead, cadmium red, cadmium mercury red, antimony orange, Permanent Red 4R, Para Red, Fire Red, p-chloro-o-nitroaniline red, Lithol Fast Scarlet G, Brilliant Fast Scarlet, Brilliant Carmine BS, Permanent Red (F2R, F4R, FRL, FRLL and F4RH), Fast Scarlet VD, Vulcan Fast Rubine B, Brilliant Scarlet G, Lithol Rubine GX, Permanent Red F5R, Brilliant Carmine 6B, Pigment Scarlet 3B, Bordeaux 5B, Toluidine Maroon, Permanent Bordeaux F2K, Helio Bordeaux BL, Bordeaux 10B, BON Maroon Light, BON Maroon Medium, Eosin Lake, Rhodamine Lake B, Rhodamine Lake Y, Alizarine Lake, Thioindigo Red B, Thioindigo Maroon, Oil Red, Quinacridone Red, Pyrazolone Red, polyazo red, Chrome Vermilion, Benzidine Orange, perynone orange, Oil Orange, cobalt blue, cerulean blue, Alkali Blue Lake, Peacock Blue Lake, Victoria Blue Lake, metal-free Phthalocyanine Blue, Phthalocyanine Blue, Fast Sky Blue, Indanthrene Blue (RS and BC), Indigo, ultramarine, Prussian blue, Anthraquinone Blue, Fast Violet B, Methyl Violet Lake, cobalt violet, manganese violet, dioxane violet, Anthraquinone Violet, Chrome Green, zinc green, chromium oxide, viridian, emerald green, Pigment Green B, Naphthol Green B, Green Gold, Acid Green Lake, Malachite Green Lake, Phthalocyanine Green, Anthraquinone Green, titanium oxide, zinc oxide, lithopone and the like. These materials can be used alone or in combination. The content of the coloring agent is from 1 to 15 % by weight and preferably from 3 to 10 % by weight based on the toner.

### Coloring Agent As Master batch

Master batch pigments, which are prepared by combining a coloring agent with a resin, can be used as the coloring agent of the toner composition of the present invention. Specific examples of the resins for use in the master batch pigments or for use in combination with master batch pigments include, but are not limited to, the modified polyester resins and the unmodified polyester resins mentioned above; styrene polymers and substituted styrene polymers such as polystyrene, poly-p-chlorostyrene and polyvinyltoluene; styrene copolymers such as styrene-p-chlorostyrene copolymers, styrene-propylene copolymers, styrene-vinyltoluene copolymers, styrene-vinylnaphthalene copolymers, styrene-methyl acrylate copolymers, styrene-ethyl acrylate copolymers, styrene-butyl acrylate copolymers, styrene-octyl acrylate copolymers, styrene-methyl methacrylate copolymers, styrene-ethyl methacrylate copolymers, styrene-butyl methacrylate copolymers, styrene-α-methyl chloromethacrylate copolymers, styrene-acrylonitrile copolymers, styrene-vinyl methyl ketone copolymers, styrene-butadiene copolymers, styrene-isoprene copolymers, styrene-acrylonitrile-indene copolymers, styrene-maleic acid copolymers and styrene-maleic acid ester copolymers; and other resins such as polymethyl methacrylate, polybutyl methacrylate, polyvinyl chloride, polyvinyl acetate, polyethylene, polypropylene, polyesters, epoxy resins, epoxy polyol resins, polyurethane resins, polyamide resins, polyvinyl butyral resins, acrylic resins, rosin, modified rosins, terpene resins, aliphatic or alicyclic hydrocarbon resins, aromatic petroleum resins, chlorinated paraffin, paraffin waxes. These resins can be used alone or in combination.

### Method of Manufacturing Master Batch

The master batch for use in the toner of the present invention is typically prepared by mixing and kneading a resin and a coloring agent upon application of high shear stress thereto. In this case, an organic solvent can be used to boost the interaction of the coloring agent with the resin. In addition, flushing methods in which an aqueous paste including a coloring agent is mixed with a resin solution of an organic solvent to transfer the coloring agent to the resin solution and then the aqueous liquid and organic solvent are separated to be removed can be preferably used because the resultant wet cake of the coloring agent can be used as it is. In this case, three-roll mills, can be preferably used for kneading the mixture upon application of high shear stress thereto.

### Releasing Agent

A release agent may be included in the toner of the present invention. Suitable release agents include known waxes.

Specific examples of the release agent include, but are not limited to, polyolefin waxes such as polyethylene waxes and polypropylene waxes; long chain hydrocarbons such as paraffin waxes and SAZOL waxes; waxes including a carbonyl group, ; rice wax and synthetic esters.

Specific examples of the waxes including a carbonyl group include, but are not limited to, polyalkane acid esters such as carnauba wax, montan waxes, trimethylolpropane tribehenate, pentaerythritol tetrabehenate, pentaerythritol diacetate dibehenate, glycerin tribehenate, and 1,18-octadecanediol distearate; polyalkanol esters such as trimellitic acid tristearyl, and distearyl maleate; polyalkylamide such as trimellitic acid tristearylamide; dialkyl ketone such as distearyl ketone . Among these materials, polyalkane acid esters are preferred.

In the present invention, the content of the releasing agent (wax) in the toner is preferably from 3 to 30 % by weight based on the entire content of the toner. When the content of the releasing agent is too small, the releasing agent is not effective to demonstrate the releasing effect, thereby losing a margin for smear protection. When the content of the releasing agent is too large, the releasing agent tends to melt at a low temperature so that the releasing agent is easily affected by thermal energy and mechanical energy. Thus, the releasing agent easily oozes from the inside of the toner during stirring in the development device and attaches to the toner regulating applicator (blade) and the image bearing member, which may lead to the occurrence of the image noise. The toner can be fixed at a low temperature when the endothermic peak of the releasing agent at temperature rising measured by a differential scanning calorimeter (DSC) ranges from 65 to 115 °C. An endothermic peak that is too low tends to degrade the fluidity. An endothermic peak that is too high tends to degrade the fixing property.

### Charge Controlling Agent

A charge controlling agent may be included in the toner of the present invention.

Specific examples of the charge controlling agent include, but are not limited to, known charge controlling agents such as Nigrosine dyes, triphenylmethane dyes, metal complex dyes including chromium, chelate compounds of molybdic acid, Rhodamine dyes, alkoxyamines, quaternary ammonium salts (including fluorine-modified quaternary ammonium salts), alkylamides, phosphor and compounds including phosphor, tungsten and compounds including tungsten, fluorine-containing activators, metal salts of salicylic acid, metal salts of salicylic acid derivatives, .

Specific examples of the marketed products of the charge controlling agents include, but are not limited to, BONTRON 03 (Nigrosine dyes), BONTRON P-51 (quaternary ammonium salt), BONTRON S-34 (metal-containing azo dye), E-82 (metal complex of oxynaphthoic acid), E-84 (metal complex of salicylic acid), and E-89 (phenolic condensation product), which are manufactured by Orient Chemical Industries Co., Ltd.; TP-302 and TP-415 (molybdenum complex of quaternary ammonium salt), which are manufactured by Hodogaya Chemical Co., Ltd.; COPY CHARGE PSY VP2038 (quaternary ammonium salt), COPY BLUE (triphenyl methane derivative), COPY CHARGE NEG VP2036 and NX VP434 (quaternary ammonium salt), which are manufactured by Hoechst AG; LRA-901, and LR-147 (boron complex), which are manufactured by Japan Carlit Co., Ltd.; copper phthalocyanine, perylene, quinacridone, azo pigments and polymers having a functional group such as a sulfonate group, a carboxyl group, a quaternary ammonium group, .

### External Additive

### Inorganic Particulate

An external additive can be added to the toner of the present invention to help improving the fluidity, developability, chargeability of the coloring agent prepared or obtained in the present invention. Inorganic particulates are suitably used as such an external additive. It is preferred for the inorganic particulate to have a primary particle diameter of from 5 nm to 2 µm, and more preferably from 5 nm to 500 nm. In addition, it is preferred that the specific surface area of such inorganic particulates measured by the BET method is from 20 to 500 m²/g. The content of such an inorganic particulate is preferably from 0.01 to 5 % by weight and particularly preferably from 0.01 to 2.0 % by weight based on the weight of a toner.

Specific examples of such inorganic particulates include, but are not limited to, silica, alumina, titanium oxide, barium titanate, magnesium titanate, calcium titanate, strontium titanate, zinc oxide, tin oxide, quartz sand, clay, mica, sand-lime, diatom earth, chromium oxide, cerium oxide, red iron oxide, antimony trioxide, magnesium oxide, complex compounds such as silicon oxide and magnesium oxide or silicon oxide and aluminum oxide, zirconium oxide, barium sulfate, barium carbonate, calcium carbonate, silicon carbide, silicon nitride, . Silica is suitably used in terms of fluidity and chargeability.

### Polymer Particulate

In addition, polymer particulates, such as polystyrene, methacrylate copolymers and acrylate copolymers, which are obtained by soap-free emulsification polymerization and suspension polymerization and dispersion polymerization, and polycondensation thermocuring resin particles, such as silicone, benzoguanamine and nylon, can be used.

### Surface Treatment of External Additive

The fluidizers (external additives) specified above can be surface-treated to improve the hydrophobic property and prevent deterioration of the fluidity characteristics and chargeability in a high humidity environment. Preferred specific examples of surface treatment agents include, but are not limited to, silane coupling agents, silyl agents, silane coupling agents having a fluorine alkyl group, organic titanate coupling agents, aluminum-based coupling agents, silicone oil, and modified-silicone oil.

### Cleaning Property Improver

As a cleaning property improver to remove a development agent remaining on an image bearing member or a primary transfer medium after transfer, stearic acid, aliphatic metal salts, for example, zinc stearate and calcium stearate, and polymer particulates manufactured by soap-free emulsification polymerization, such as polymethyl methacrylate particulates and polystyrene particulates, can be used. Such polymer particulates preferably have a relatively sharp particle size distribution and a volume average particle size of from 0.01 to 1 µm.

### Method of Manufacturing Toner

A preferable example method of manufacturing the toner of the present invention is described below but the method of manufacturing the toner of the present invention is not limited thereto.

The method of manufacturing the toner of the present invention includes at least a granulation process in which at least a polyester resin, a coloring agent and a releasing agent are dissolved or dispersed in an organic solvent and thereafter the lysate or dispersed material is dispersed in an aqueous medium to granulate core particles and an attachment process of particulates to the core particles in which an aqueous liquid dispersion in which at least vinyl based copolymer resin particulates are dispersed is added to the core particles.

The method is described in detail below.

### Granulation of Core Particles

### Organic Solvent

The organic solvent that dissolves or disperses a toner composition formed of a polyester resin, a coloring agent and a releasing agent preferably has a Hansen dissolution parameter of not greater than 19.5. The Hansen dissolution parameter is described in, for example, Section VI I in Volume 2 of "Polymer Handbook" 4th edition published by Wiley-Interscience. Considering that the solvent is removed later, the boiling point of the solvent is preferably lower than 100 °C. Specific examples thereof include, but are not limited to, toluene, xylene, benzene, carbon tetrachloride, methylene chloride, 1,2-dichloroethane, 1,1,2-trichloroethane, trichloroethylene, chloroform, monochlorobenzene, dichloroethylidene, methyl acetate, ethyl acetate, methylethyl ketone and methylisobuthyl ketone. These can be used alone or in combination. Among these, ester based solvents such as methyl acetate and ethyl acetate, aromatic based solvent such as toluene and xylene, and halogenized hydrocarbons such as methylene chloride, 1,2-dichloroethane, chloroform and carbon tetrachloride are especially preferred. The polyester resin, the coloring agent and the releasing agent can be simultaneously dissolved or dispersed but typically dissolved or dispersed in separate occasions. The organic solvent to dissolve or disperse each of the polyester resin, the coloring agent and the releasing agent can be the same or different but using the same organic solvent is preferable considering the subsequent solvent treatment.

### Dissolution or Dispersion of Polyester Resin

The resin density in the liquid dissolution or dispersion of a polyester resin is preferably from about 40 to 80 % by weight. A resin density that is too high tends to make dissolution or dispersion difficult and the viscosity high so that handling liquid dissolution or dispersion is difficult. When the resin density is too low, the amount of produced toner tends to decrease. When a modified polyester resin having an isocyanate group at its end is mixed with a polyester resin, the modified polyester resin and the polyester resin can be mixed in the same liquid dissolution or dispersion or manufactured separately in different liquid dissolution or dispersion.

### Considering the solubility and the viscosity thereof, it is preferable to separately prepare different liquid dissolution or dispersion. Dissolution or Dispersion of Coloring Agent

The coloring agent can be separately dissolved or dispersed or mixed with the liquid dissolution or dispersion of the polyester resin. If desired, a dispersion helping agent or a polyester resin can be added or the master batch specified above can also be used. Dissolution or Dispersion of Infrared Absorption Agent

The infrared absorption agent can be solely dissolved or dispersed or mixed with the solution or liquid dispersion of the polyester resin. The infrared absorption agent can be used alone or in combination. A dispersion helping agent or a polyester resin can be optionally added to the infrared absorption agent and the infrared absorption agent can be mixed in the master batch specified above and used as the master batch.

### Dissolution or Dispersion of Releasing Agent

When a wax is dissolved or dispersed as the releasing agent and an organic solvent in which the wax is not soluble is used, the resultant is used as a liquid dispersion. Such a liquid dispersion is prepared by a typical method, in which an organic solvent and a wax are mixed followed by dispersion treatment by a dispersion device such as a bead mill. Alternatively, after mixing an organic solvent and a wax, the wax is heated to the melting point thereof and cooled down while being stirred. Thereafter, the mixture is dispersed by a dispersion device such as a bead mill. In this method, the dispersion time may be reduced. Furthermore, several kinds of waxes can be mixed for use and a dispersion improving agent or a polyester resin can be optionally added.

### Aqueous Medium

Suitable aqueous media for use in the present invention include water, and mixtures of water with a solvent which can be mixed with water. Furthermore, the organic solvent mentioned above for use in the liquid dissolution or dispersion having a Hansen dissolution parameter of not greater than 19.5 can be mixed. When such an organic solvent is added to water in an amount close to the saturation amount, the emulsification or dispersion stability of the oil phase added to the aqueous medium can be improved. Specific examples of such a solvent include, but are not limited to, alcohols (e.g., methanol, isopropanol and ethylene glycol), dimethylformamide, tetrahydrofuran, cellosolves (e.g., methyl cellosolve), lower ketones (e.g., acetone and methyl ethyl ketone). The amount of an aqueous medium is normally from 50 to 2,000 parts by weight and preferably from 100 to 1,000 parts by weight based on 100 parts by weight of a toner composition. When the amount of an aqueous medium is too small, the dispersion stability of a toner composition is degraded so that toner particles having a desired particle diameter are not obtained. An amount of an aqueous medium that is excessively large is not preferred in terms of economy.

### Inorganic Dispersion Agent and Organic Resin Particulate

The lysate or dispersion material of the toner composition mentioned above is preferably dispersed in an aqueous medium in which an inorganic dispersion agent or organic resin particulates are preliminarily dispersed to have a sharp particle size distribution and stabilize the dispersion. Specific examples of the inorganic dispersion agent include, but are not limited to, tricalcium phosphate, calcium carbonate, titanium oxide, colloidal silica and hydroxyapatite. There is no specific limit to selection of resins that form resin particulates as long as the resin can form a dispersion body in an aqueous medium. A dispersion body having fine spherical resin particulates is preferred. Any thermoplastic resins or thermocuring resins can be used as resin particulates. Specific examples thereof include, but are not limited to, vinyl based resins, polyurethane resins, epoxy resins, polyester resins, polyamide resins, polyimide resins, silicon based resins, phenol resins, melamine resins, urea resins, aniline resins, ionomer resins, and polycarbonate resins. These resins can be used alone or in combination. Among these, vinyl resins, polyurethane resins, epoxy resins and polyester resins and their combinational use are preferred in terms that a dispersion body having fine spherical resin particulates is easy to obtain. Method of Dispersing Organic Resin Particulate in Aqueous Medium

There is no specific limit to the method of preparing an aqueous liquid dispersion of resin particulates from a resin. For example, the following methods of (a) to (h) can be used.
(a) A method of manufacturing an aqueous liquid dispersion of resin particulate directly from the polymerization reaction by a suspension polymerization method, an emulsification polymerization method, a seed polymerization method or a dispersion polymerization method from a monomer as the start material in the case of a vinyl based resin.
(b) A method of manufacturing an aqueous liquid dispersion of resin particulates by: dispersing a precursor (monomer, oligomer, ) or its solvent solution under the presence of a suitable dispersion agent; and curing the resultant by heating and/or adding a curing agent in the case of a polyaddition or polycondensation resin such as a polyester resin, a polyurethane resin and an epoxy resin.
(c) In the case of a polyaddition or polycondensation resin such as a polyester resin, a polyurethane resin and an epoxy resin, a method of manufacturing an aqueous liquid dispersion of resin particulates by dissolving a suitable emulsification agent in a precursor (monomer, oligomer, ) or its solvent solution (liquid is preferred, e.g., liquidized by heating) followed by adding water for phase change.
(d) A method of manufacturing an aqueous liquid dispersion of resin particulates by: fine-pulverizing resins preliminarily manufactured by a polymer reaction (addition polymerization, ring scission polymerization, polyaddition, addition condensation, polycondensation, ) with a fine grinding mill of a mechanical rotation type or jet type; classifying the resultant; and dispersing the obtained resin particulates in water under the presence of a suitable dispersion agent.
(e) A method of manufacturing an aqueous liquid dispersion of resin particulates by: spraying in the form of a fine liquid mist a resin solution in which resins preliminarily manufactured by a polymer reaction (addition polymerization, ring scission polymerization, polyaddition, addition condensation, polycondensation, ) are dissolved in a solvent; and dispersing the obtained resin particulates in water under the presence of a suitable dispersion agent.
(f) A method of manufacturing an aqueous liquid dispersion of resin particulates by: precipitating resin particulates by adding a solvent to a resin solution in which resins preliminarily manufactured by a polymer reaction (addition polymerization, ring scission polymerization, polyaddition, addition condensation, polycondensation, ) are dissolved in another solvent or cooling the resin solution preliminarily prepared by heating and dissolving in a solvent; removing the solvent to obtain the resin particulates; and dispersing the obtained resin particulates in water under the presence of a suitable dispersion agent.
(g) A method of manufacturing an aqueous liquid dispersion of resin particulates by: dispersing in an aqueous medium a resin solution in which resins preliminarily manufactured by a polymer reaction (addition polymerization, ring scission polymerization, polyaddition, addition condensation, polycondensation, ) are dissolved in a solvent under the presence of a suitable dispersion agent; and removing the solvent by heating, reducing pressure, etc.
(h) A method of manufacturing an aqueous liquid dispersion of resin particulates by: dissolving a suitable emulsification agent in a resin solution in which resins preliminarily manufactured by a polymer reaction (addition polymerization, ring scission polymerization, polyaddition, addition condensation, polycondensation, ) are dissolved in a solvent; and adding water for phase change.

### Surface Active Agent

To emulsify and/or disperse an oil phase containing a toner composition in an aqueous medium, a surface active agent can be used, if desired. Specific examples of the surface active agents include, but are not limited to, anionic dispersion agents, for example, alkylbenzene sulfonic acid salts, α-olefin sulfonic acid salts, and phosphoric acid salts; cationic dispersion agents, for example, amine salts (e.g., alkyl amine salts, aminoalcohol fatty acid derivatives, polyamine fatty acid derivatives and imidazoline), and quaternary ammonium salts (e.g., alkyltrimethyl ammonium salts, dialkyldimethyl ammonium salts, alkyldimethyl benzyl ammonium salts, pyridinium salts, alkyl isoquinolinium salts and benzethonium chloride); nonionic dispersion agents, for example, fatty acid amide derivatives, polyhydric alcohol derivatives; and ampholytic dispersion agents, for example, alanine, dodecyldi(aminoethyl)glycin, di(octylaminoethyle)glycin, and N-alkyl-N,N-dimethylammonium betaine.

An extremely small amount of a surface active agent having a fluoroalkyl group is effective for a good dispersion. Preferred specific examples of the anionic surface active agents having a fluoroalkyl group include, but are not limited to, fluoroalkyl carboxylic acids having from 2 to 10 carbon atoms and their metal salts, disodium perfluorooctanesulfonylglutamate, sodium 3-{omega-fluoroalkyl(C6-C11)oxy}-1-alkyl(C3-C4) sulfonate, sodium 3-{omega-fluoroalkanoyl(C6-C8)-N-ethylamino}-1-propanesulfonate, fluoroalkyl(C11-C20) carboxylic acids and their metal salts, perfluoroalkylcarboxylic acids and their metal salts, perfluoroalkyl(C4-C12)sulfonate and their metal salts, perfluorooctanesulfonic acid diethanol amides, N-propyl-N-(2-hydroxyethyl)perfluorooctanesulfone amide, perfluoroalkyl(C6-C10) sulfoneamidepropyltrimethylammonium salts, salts of perfluoroalkyl(C6-C10)-N-ethylsulfonyl glycin, monoperfluoroalkyl(C6-C16)ethylphosphates, . Specific examples of the cationic surface active agents having a fluoroalkyl group include, but are not limited to, primary and secondary aliphatic amino acids, secondary amino acids, aliphatic quaternary ammonium salts (for example, perfluoroalkyl(C6-C10)sulfoneamidepropyltrimethyl ammonium salts), benzalkonium salts, benzetonium chloride, pyridinium salts, and imidazolinium salts.

### Protective Colloid

It is possible to stabilize liquid droplet dispersion in an aqueous medium using a polymeric protection colloid. Specific examples of such polymeric protection colloids include, but are not limited to, polymers and copolymers prepared using monomers, for example, acids (e.g., acrylic acid, methacrylic acid, α-cyanoacrylic acid, α-cyanomethacrylic acid, itaconic acid, crotonic acid, fumaric acid, maleic acid and maleic anhydride), acrylic monomers having a hydroxyl group (e.g., β-hydroxyethyl acrylate, β-hydroxyethyl methacrylate, β-hydroxypropyl acrylate, β-hydroxypropyl methacrylate, γ-hydroxypropyl acrylate, γ-hydroxypropyl methacrylate, 3-chloro-2-hydroxypropyl acrylate, 3-chloro-2-hydroxypropyl methacrylate, diethyleneglycolmonoacrylic acid esters, diethyleneglycolmonomethacrylic acid esters, glycerinmonoacrylic acid esters, N-methylolacrylamide and N-methylolmethacrylamide), vinyl alcohol and its ethers (e.g., vinyl methyl ether, vinyl ethyl ether and vinyl propyl ether), esters of vinyl alcohol with a compound having a carboxyl group (i.e., vinyl acetate, vinyl propionate and vinyl butyrate); acrylic amides (e.g, acrylamide, methacrylamide and diacetoneacrylamide) and their methylol compounds, acid chlorides (e.g., acrylic acid chloride and methacrylic acid chloride), and monomers having a nitrogen atom or a heterocyclic ring having a nitrogen atom (e.g., vinyl pyridine, vinyl pyrrolidone, vinyl imidazole and ethylene imine).

In addition, polymers, for example, polyoxyethylene compounds (e.g., polyoxyethylene, polyoxypropylene, polyoxyethylenealkyl amines, polyoxypropylenealkyl amines, polyoxyethylenealkyl amides, polyoxypropylenealkyl amides, polyoxyethylene nonylphenyl ethers, polyoxyethylene laurylphenyl ethers, polyoxyethylene stearylphenyl esters, and polyoxyethylene nonylphenyl esters), and cellulose compounds, for example, methyl cellulose, hydroxyethyl cellulose and hydroxypropyl cellulose, can also be used as the polymeric protective colloid. When compounds, for example, calcium phosphate, which are soluble in an acid or alkali, are used as a dispersion stabilizer, it is possible to dissolve the calcium phosphate by adding an acid, for example, hydrochloric acid, followed by washing of the resultant particles with water, to remove the calcium phosphate from particulates. In addition, a zymolytic method can be used to remove such compounds. Such a dispersion agent may remain on the surface of toner particles. However, it is preferred to wash and remove the dispersion agent in terms of the charging property of toner particles. Dispersion Method

There is no particular limit to the dispersion method. Low speed shearing methods, high speed shearing methods, friction methods, high pressure jet methods, ultrasonic methods, , can preferably be used. Among these methods, high speed shearing methods are more preferable because particles having a particle diameter of from 2 to 20 µm can be easily prepared. When a high speed shearing type dispersion machine is used, there is no particular limit to the rotation speed thereof, but the rotation speed is typically from 1, 000 to 30,000 rpm, and preferably from 5,000 to 20,000 rpm. The temperature during the dispersion process is typically from 0 to 150 ° C (under pressure), and preferably from 20 to 80 ° C.

### Solvent Removal

Any known methods can be used to remove organic solvents from the obtained emulsified dispersion body.

For example, a method can be employed in which the system is gradually heated under normal pressure or with a reduced pressure to completely evaporate and remove organic solvent in the droplets.

### Attachment Process of Particulate

The process of attaching particulates mainly formed of a vinyl based copolymer resin to the core particles mainly formed of a polyester resin is described. In this process, using an aqueous liquid dispersion in which at least vinyl based copolymer particulates are dispersed is suitable. This liquid dispersion is easily manufactured by a typical emulsification polymerization method and can be used in the attachment process as it is. To stabilize the core particles and the particulates in some degree, a surface active agent can be suitably added. A preferable timing of adding the particulates is after removal of organic solvent.

To conduct attachment more efficiently, sodium hydroxide or hydrochloric acid can be added to adjust PH in the attachment process. Also, mono-, di- or tri-metal salts can be used as an agglomeration agent. Specific examples of the mono-valent metals include, but are not limited to, lithium, potassium and sodium. Specific examples of the divalent metals include, but are not limited to, calcium and magnesium. A specific example of the trivalent metals includes, but is not limited to, aluminum. Specific examples of anions that form the salts include, but are not limited to, chloride ion, bromide ion, iodine ion, carbonate ion and sulfate ion. In addition, attachment can be accelerated by heating. The particulates can be attached to the core particles at a temperature lower or higher than the glass transition temperature of the particulates. When the particulates are attached at a temperature around or lower than the glass transition temperature, agglomeration and/or adhesion of the particulates hardly occur in some cases. Therefore, it is preferred to heat the particulates thereafter to a higher temperature to accelerate agglomeration and/or adhesion and coverage of the core particles and make the surface of the shell portion uniform. The heating temperature and the heating time are suitably selected in terms of the adjustment of the uniformity of the surface and the sphericity of toner particles.

### Elongation and/or Cross Linking Reaction

When a modified polyester resin having an isocyanate group at its end and an amine reactive therewith are added to introduce a modified polyester resin having a urethane and/or a urea linkage, the amine can be mixed in an oil phase before a toner component is dispersed in an aqueous medium or added to the aqueous medium. The reaction time is determined depending on the isocyanate group structure included in a polyester prepolymer and the reactivity thereof with the added amine and is typically from 1 minute to 40 hours and preferably from 1 to 24 hours. The reaction temperature is from 0 to 150 °C and preferably from 20 to 98 °C. This reaction can be conducted before, during, or after the particulate attachment process described above. Any known catalyst can be used in the elongation reaction and/or cross linking reaction, if desired.

### Washing and Drying Process

Known technologies are used in the process of washing and drying colored particles dispersed in an aqueous medium. That is, after solid and liquid of an aqueous medium are separated by a centrifugal or a filter press to obtain a toner cake, the obtained cake is re-dispersed in de-ionized water at room temperature to about 40 ° C. Subsequent to optional pH adjustment by an acid or an alkali, the resultant is subject to the solid and liquid separation treatment again. This cycle is repeated several times to remove impurities and the active surface agent. Thereafter, the resultant is dried by an air stream drier, a circulation drier, a reduced pressure drier, a vibration flow drier, to obtain colored particle powder. The particulate component of the colored particle can be removed by a centrifugal or a known classifier can be optionally used after drying to obtain toner having a desired particle size distribution.

### External Addition Treatment

The thus prepared colored particles powder after drying can be mixed with other particles such as the charge control agent particulates and fluidizing agent particulates. Such particles can be fixed on the toner particles by applying a mechanical impact thereto to integrate the particles into toner particles. Thus, the other particles can be prevented from being detached from the toner particles. Specific examples of such mechanical impact application methods include, but are not limited to, methods in which a mixture is mixed by a blade rotating at a high speed and methods in which a mixture is put into a jet air to collide the particles against each other or a collision plate.

Specific examples of such mechanical impact applicators include, but are not limited to, ONG MILL (manufactured by Hosokawa Micron Co., Ltd.), modified I TYPE MILL (manufactured by Nippon Pneumatic Mfg. Co., Ltd.) in which the pressure of pulverization air is reduced, HYBRIDIZATION SYSTEM (manufactured by Nara Machine Co., Ltd.), KRYPTRON SYSTEM (manufactured by Kawasaki Heavy Industries, Ltd.), automatic mortars, .

### Fixing Helping Particle

There is no specific limit to selection of resins that form fixing helping particulates as long as the resin can form a dispersion body in an aqueous medium. A dispersion body having fine spherical resin particulates is preferred. Any thermoplastic resins or thermocuring resins can be used as resin particulates. Specific examples thereof include, but are not limited to, vinyl based resins, polyurethane resins, epoxy resins, polyester resins, polyamide resins, polyimide resins, silicon based resins, phenol resins, melamine resins, urea resins, aniline resins, ionomer resins, and polycarbonate resins. These resins can be used alone or in combination. Among these, vinyl resins, polyurethane resins, epoxy resins and polyester resins and their combinational use are preferred in terms that a dispersion body having fine spherical resin particulates is easy to obtain.

There is no specific limit to the infrared absorption agent containing the fixing helping particle as long as the infrared absorption agent is transparent or close to transparent. For example, metal oxide ultra fine particulates can be used as the infrared absorption agent. These particles may contain organic components. How a metal oxide or an organic component is contained is not specifically limited but a state in which a metal oxide is set in the center and an organic component covers around the metal oxide is preferred. Specific examples of the metal components contained in the metal oxides include, but are not limited to, Cu, Zn, In, Si, Ge, Sn, Fe, Co, Ni, Ru, Rh, Os, Ir, V, Cr, Mn, Y, Ti, Zr, Nb, Mo, Ca, Ba, Sb, Al, Mg, and Bi. Such metal components are preferably metal components deriving from the metal organic compound as the manufacturing material of the metal oxide ultra fine particulate. Specific examples of the metal oxides include, but are not limited to, Al₂O₃, ZnO, In₂O₃, SnO₂, and Sb₂O₃. These metal oxides are used alone or in combination. When used in combination, a mixture of these metal oxides or complex metal oxides thereof is suitable. Preferred specific examples of the complex metal oxides include, but are not limited to, metal oxides containing In₂O₃ and SnO₂. A metal oxide substantially formed of In₂O₃ and SnO₂ is more preferred. To be specific, ITO is preferred in which SnO₂ is doped with In₂O₃. The content of the infrared absorption agent in the fixing helping agent is preferably from about 1 to about 50 % by weight and more preferably from about 1 to 30 parts by weight. The fixing helping particle can be prepared by mixing each component. For example, particular amounts of metal oxide ultra fine particulates, an organic solvent and a resin are prepared and the metal oxide ultra fine particulates and the resin are added to the organic solvent. Thereafter the system is sufficiently stirred by a stirrer followed by removing the organic solvent and drying the resultant.

### Development Agent

The toner for use in the present invention can be used as a two component development agent. In such a two component development agent, the toner is used as a mixture with a carrier and the ratio of the carrier to the toner in the development agent is preferably from 1 to 10 parts by weight based on 100 parts by weight of the carrier. Known material such as iron powder, ferrite powder, magnetite powder and magnetic resin carrier having a particle diameter of from about 20 to about 200 µm can be used the magnetic carrier. In addition, specific examples of such resins to be coated on the carriers include, but are not limited to, amino resins such as urea-formaldehyde resins, melamine resins, benzoguanamine resins, urea resins, and polyamide resins, and epoxy resins. In addition, polyvinyl or polyvinylidene resins such as acrylic resins, polymethylmethacrylate resins, polyacrylonitirile resins, polyvinyl acetate resins, polyvinyl alcohol resins, polyvinyl butyral resins, polystyrene resins, styrene-acrylic copolymers, halogenated olefin resins such as polyvinyl chloride resins, polyester resins such as polyethyleneterephthalate resins and polybutyleneterephthalate resins, polycarbonate resins, polyethylene resins, polyvinyl fluoride resins, polyvinylidene fluoride resins, polytrifluoroethylene resins, polyhexafluoropropylene resins, vinylidenefluoride-acrylate copolymers, vinylidenefluoride-vinylfluoride copolymers, fluoroterpolymers such as terpolymer of tetrafluoroethylene, vinylidenefluoride and other monomers including no fluorine atom, and silicone resins can be used.

If desired, an electroconductive powder may be included in the coating resin. Specific examples of such electroconductive powders include, but not limited to, metal powder, carbon black, titanium oxides, tin oxides, and zinc oxides. The average particle diameter of such electroconductive powders is preferably not greater than 1 µm. When the particle diameter is greater than 1 µm, controlling the resistance tends to be difficult. The toner for use in the present invention can also be used as a magnetic toner or a non-magnetic toner of a single component in which no carrier is used.

An image forming apparatus which can be used in the method of the present invention is described next.

Fig. 1 is a schematic diagram illustrating an example of the image forming apparatus. An image bearing member 1 is charged by a charging device 2 and thereafter irradiated with light by an irradiating device 3 so that a latent electrostatic image is written on the image bearing member 1. A bias is applied to a development roller 40 contained in a development unit 4 and the image bearing member 1. The written latent electrostatic image is developed and visualized at the contact point with a development agent 44 supplied from a supply roller 41 to a development roller 40 followed by regulation of the toner layer on the development roller 40 by a regulating blade 43. The development agent 44 used for development and visualization of the latent electrostatic image is temporarily transferred to an intermediate transfer material 44 and then to a recording medium 9 via a supporting roller 10 and a transfer roller 5 and fixed thereon by a fixing device. An extremely small amount of the development agent 44 passes through the intermediate transfer material 8 and remains on the image bearing member 1. The toner remaining on the surface of the image bearing member 1 after transfer is collected by a cleaning device 7 and discarded.

The development portion is described next.

Fig. 2 is a schematic diagram illustrating an example of the development unit (process cartridge) 4. The development agent (toner) 44 in the toner supply portion in the toner container is transferred to the nip portion of the development roller 40 where the development roller 40 nips the development agent 44 with the supply roller 41. Thereafter, the amount of the toner on the development roller 40 is regulated by the regulating blade 43 to form a thin layer of the toner on the development roller 40. In addition, the toner is abraded at the nip portion formed between the supply roller 41 and the development roller 40 and between the regulating blade 43 and the development roller 40 to have a suitable amount of charge. In the structure having no cleaning device, the amount of charge of the toner is significantly away from a suitable range and therefore, the toner collected by the development roller is sufficiently scraped and removed by the supply roller.

The non-contact fixing device is described below.

Fig. 3 is a schematic diagram illustrating an example of the non-contact fixing device for use in the present invention. Light flashes on a recording medium 102 such as paper transferred by a transfer belt 101 when the recording medium 102 passes through a flash fixing portion 103. Thus, the toner on the recording medium 102 such as paper is melted and fixed thereon. In addition, the gloss of the image on the recording medium 102 is improved by providing a smoothing mechanism 104 for smoothing the toner surface on the downstream side of the toner fixing.

A xenon lamp having emission spectrum peaks at least in the oscillation wavelength ranges of from 810 to 840nm and from 900 to 980 nm can be used as the light source of the flash fixing portion. Process Cartridge

The development agent for use in the present invention can be used in an image forming apparatus having a process cartridge as illustrated in Fig. 4.

In the present invention, the process cartridge is formed of the image bearing member described above and at leat one optional devices described above, such as the charging device, the development device and the cleaning device, and structured to be detachably attachable to the main body of an image forming apparatus such as a photocopier and a printer.

The process cartridge illustrated in Fig. 4 has an image bearing member, a development device, a charging device, and a cleaning device. First, the image bearing member is rotationally driven at a predetermined circumference speed. The image bearing member is uniformly charged negatively or positively to a predetermined voltage at its surface by the charging device while in the rotation process. Then, the image bearing member is irradiated with slit irradiation or a laser beam scanning irradiation by an irradiation device according to obtained image information. Thus, a latent electrostatic image is formed on the surface of the image bearing member and developed with toner by the development device. The developed toner image is transferred to a transfer medium which is fed from a paper feeder to the portion between the image bearing member and the transfer device in synchronization with the rotation of the image bearing member. The transfer medium having the toner image thereon is separated from the surface of the image bearing member, introduced into the fixing device where the toner image is fixed on the transfer medium and then discharged outside as an output (a photocopy or a print). The surface of the image bearing member after the image transfer is cleared of residual toner remaining thereon by the cleaning device, discharged and then ready for the next image formation cycle.

Physical properties of the colored particles, the fixing helping particulate, and the toner and the number average molecular weight (Mn), and the weight average molecular weight (Mw) of the polyester are measured as follows.

### Measuring Method

### Particle Diameter

The method of measuring the particle size distribution of the toner particles is described next.

The particle size distribution of the colored particles and the toner can be measured by Coulter counter method. For example, Coulter Counter TA-II and Coulter Multisizer II (both are manufactured by Beckman Coulter, Inc.) can be used as the measuring equipment. The measuring method is as follows:

First, add 0.1 to 5 ml of a surface active agent (preferably alkyl benzene sulfonate salt) as a dispersant to 100 to 150 ml of an electrolytic aqueous solution, which is about 1 % NaCl aqueous solution prepared by using primary NaCl and pure water, for example, ISOTON-II (manufactured by Beckman Coulter, Inc.) can be used; Add 2 to 20 mg of a measuring sample of solidified toner to the electrolytic aqueous solution; Conduct dispersion treatment for the electrolytic aqueous solution in which the measuring sample is dispersed for about 1 to 3 minutes by an ultrasonic dispersion device; Measure the volume and the number of the colored particles and the toner by the equipment mentioned above with an aperture of 100 µm; and calculate the volume distribution and the number distribution. The weight average particle diameter (Dv) and the number average particle diameter (Dn) of the colored particles or the toner can be obtained based on the obtained distributions.

The whole range is a particle diameter of from 2.00 to less than 40.30 µm and the number of the channels is 13. Each channel is: from 2.00 to not greater than 2.52 µm; from 2.52 to not greater than 3.17 µm; from 3.17 to not greater than 4.00 µm; from 4.00 to not greater than 5.04 µm; from 5.04 to not greater than 6.35 µm; from 6.35 to not greater than 8.00 µm; from 8.00 to not greater than 10.08 µm; from 10.08 to not greater than 12.70 µ m; from 12.70 to not greater than 16.00 µm, from 16.00 to not greater than 20.20 µm; from 20.20 to not greater than 25.40 µ m; from 25.40 to not greater than 32.00 µm; and from 32.00 to less than 40.30 µm.

The measuring method of the particle size distribution of particles such as the fixing helping particle having a particle diameter of from 0.1 to 2 µm is performed by using a laser diffraction diffusion method particle size distribution measuring device Microtrack MT 3300 II (manufactured by Nikkiso Co., Ltd.). The volume and the number of particles are measured to calculate the volume distribution and the number distribution. According to the obtained distribution, the volume average particle diameter (Dv) and the number average particle diameter (Dp) of the particle are obtained.

Specifically, particle sample is diluted until the solid portion density is from 1 to 5 % by weight and subject to a two minute treatment by an ultrasonic dispersion device (ultrasonic homogeniger, manufactured by Nippon Seiki Co., Ltd.). Thereafter, the agglomeration of particles is unstiffened followed by measurement for 30 seconds.

### Particulate Diameter

The particle diameter of the vinyl based copolymer particulate can be measured using a dispersion body as it is by a laser diffraction and diffusion method particle size distribution measuring device such as LA-920 (manufactured by Horiba Ltd.) or UPA-EX150 (manufactured by Nikkiso Co., Ltd.).

### Average Circularity

An optical detection method can be used for measuring particle forms in which particle images are optically detected by a charge coupled device (CCD) camera while a suspension containing particles passes through an imaging detective portion having a plate form. The average circularity of the particle is determined by dividing the circumferential length of the circle having the area equal to a projected toner area with the circumferential length of the projected toner area. This value is a value measured by a flow type particle image analyzer FPIA-2100 as the average circularity. The specific procedure for obtaining the average circularity is as follows:
(1) A surface active agent serving as a dispersion agent, preferably 0.1 to 5 ml of an alkylbenzenesulfonic acid salt, is added to 100 to 150 ml of water from which solid impurities have been preliminarily removed;
(2) About 0.1 to 0.5 g of a sample to be measured is added into the mixture prepared in (1);
(3) The mixture prepared in (2) is subjected to an ultrasonic dispersion treatment for about 1 to 3 minutes such that the concentration of the particles is 3, 000 to 10, 000 particles per micro litter; and
(4) The form and average particle diameter distribution of the sample are measured by the instrument mentioned above.

The average circularity of particles having a particle diameter of from 0.1 to 2 µm is measured by observation by a scanning electron microscope (SEM). Specifically, a value is obtained by dividing the circumference length of a circle obtained by the corresponding diameter using a photograph of a magnifying power of 1,000 with the circumference length of one particle and this value is obtained for 50 particles. Then, the average is calculated and used as the average circularity.

### Glass Transition Temperature

The glass transition temperature (Tg) of the polyester resin and the vinyl based copolymer resin can be measured by using, for example, a differential scanning calorimeter (e.g., DSC-6220R, manufactured by Seiko Instruments Inc.) as follows: Heat a sample from room temperature to 150 °C at a temperature rise speed of 10 °C/min; Leave the sample at 150 °C for 10 minutes; Cool down the sample at a temperature fall speed of 10 °C/min; Heat the sample again from 20 to 150 °C at a temperature rise speed of 10 °C/min; and obtain the glass transition temperature as the shoulder value between the base line below the glass transition temperature and the endothermic peak.

### Method of Measuring Softening Point (Tm)

Weigh 1.0 g of a sample using a flow tester (CFT-500, manufactured by Shimadzu Corporation) and measure the sample under the following conditions:
Die: height: 1.0 mm; Φ: 0.5 mm
Temperature rising speed: 3.0 °C/min
Preliminary heating time: 180 seconds
Load: 30 Kg
Measuring temperature range: 60 to 160 °C

The softening point (Tm) is determined as the temperature when a half of the sample is effused.

### GPC Analysis Method

The molecular weights (Mn and Mw) of the polyester resin manufactured in Examples described later are measured under the following conditions by typical Gel permeation chromatography (GPC). · Device: HLC-8220 (manufactured by Tosoh Corporation)
Column: TsKgel SuperHZM-M × 3
· Temperature: 40 °C
· Solvent: Tetrahydrofuran (THF)
· Current speed: 0.35 ml/min.
· Density of sample: 0.05 to 0.6 weight %
· Amount of poured sample: 0.01 m1
· Detector: UV (230 nm)

The number average molecular weight (Mn) and the weight average molecular weight (Mw) of the toner resin are calculated from the molecular distribution measured under the condition specified above by using the molecular weight calibration curve made based on monodispersity polystyrene standard sample. 10 samples having a range of from 5.8 × 10² to 7.5 × 10⁶ are used as the monodispersity polystyrene standard sample.

Manufacturing Examples of the infrared absorption agent are described below.

### Manufacturing Example of Infrared absorption agent B (Indolenine Compound)

2.7 parts by weight of 4,5-benzo-1-(2-methoxyethyl)-3,3-dimethyl-2-methylene indoline and 0.8 parts by weight of 2-chloro-1-formyl-3-hydroxymethylene cyclohexane are boiled up in 4.0 parts by weight of acetic anhydride for one hour while cooled down with reflux and then cooled down to room temperature. The reaction liquid is suction-filtrated to remove undissolved impurities. The reaction liquid is infused to 4.0 parts by weight of water in which 0.5 parts of tetrafluoro sodium borate are dissolved and obtained dissipated crystal is suction-filtrated to recrystalize by 2.0 parts by weight of DMF. Subsequent to washing by 2.0 parts by weight of methanol and drying, 2.5 parts of [Infrared absorption agent (indolenine compound) B] represented by the following Chemical structure (1). The maximum absorption wavelength of this [Infrared absorption agent B] is 820 nm.

### Manufacturing Example of Infrared absorption agent C (Aminium Compound)

1.38 g of N,N,N',N'-tetrakis(p-dibutyl aminophenyl)-p-phenylnene diamine is dissolved in ethyl acetate and 6 ml of acetnitrile and a solution in which 0.22 g of sodium perchlorate and 1.13 g of ammonium salt of ferric complex salt of 1,3-diaminopropane tetraacetate are dissolved in 6ml of water are added. The resultant is stirred at 30 °C for 6 hours. The reaction mixture is washed by water and condensed under a reduced pressure and n-heptane is added thereto to precipitate a crystal. The precipitated crystal is filtered and dried to obtain green powder of the [Infrared absorption agent C (aminium compound)] having the following Chemical structure (2). The maximum absorption wavelength of this [Infrared absorption agent C] is 950 nm.

### Ultra Fine Particulate D Having Infrared Absorption Power Added to Fixing Helping Particle

Complex ultrafine particulate (ITO, manufactured by Tomoe Works Co., Ltd.) in which SnO₂ is doped in In₂O₃ is used. The content of SnO₂ ([Sn/ (Sn + In)]) in the complex ultrafine particulate (reduced quantity in metal) is 5 % by weight in metal in reduced quantity. The density of the metal oxide in the complex ultrafine particulate is 90 % by weight. The complex ultrafine particulate has a metal oxide in the center and an organic compound covering the metal oxide and the average particle diameter of the complex ultrafine particulate is 20 nm.

Having generally described preferred embodiments of this invention, further understanding can be obtained by reference to certain specific examples which are provided herein for the purpose of illustration only and are not intended to be limiting. In the descriptions in the following examples, the numbers represent weight ratios in parts, unless otherwise specified.

### EXAMPLES

The present invention is specifically described in detail with reference to Examples but not limited thereto.

### Synthesis of Polyester

### Polyester 1

The following components are placed in a container equipped with a condenser, a stirrer and a nitrogen introducing tube to conduct a reaction at 230 °C at normal pressure for 8 hours followed by another reaction for 5 hours with a reduced pressure of 10 to 15 mmHg and 26 parts by weight of trimellitic anhydride is added to the reaction container to conduct a reaction at 180 °C at normal pressure for 2 hours to obtain [Polyester 1].

| | |
|---|---|
| Adduct of bisphenol A with 2 mole of ethylene oxide | 553 parts |
| Adduct of bisphenol A with 2 mole of propylene oxide | 196 parts |
| Terephthalic acid | 220 parts |
| Adipic acid | 45 parts |
| Dibutyl tin oxide | 2 parts |

[Polyester 1] has a number average molecular weight of 2,200, a weight average molecular weight of 5,600, a glass transition temperature of 43 °C, and an acid value of 13 mgKOH/g.

### Synthesis of Vinyl Based Copolymer Resin Particulate Vinyl Based Copolymer Resin Particulate S-1

1.6 parts by weight of dodecyl sodium sulfate and 492 parts by weight of deionized water are placed in a reaction container equipped with a condenser, a stirrer and a nitrogen introducing tube and heated to 80 °C. A solution in which 2.5 parts by weight of KPS (potassium peroxodisulfate) as a polymerization initiator is dissolved in 100 parts by weight of deionized water is added to the reaction container and 15 minutes later, a liquid mixture of a monomer composition of 152 parts by weight of styrene monomer, 38 parts by weight of butyl acrylate, 10 parts by weight of methacrylic acid and 3.5 parts by weight of NOM (n-octylmercaptan) as a molecular weight control agent is dripped to the reaction container in 90 minutes. Thereafter, the reaction system is maintained at 80 °C for 60 minutes.

Subsequent to cooling down, a liquid dispersion of [Vinyl based copolymer resin particulate S-1] is obtained. The particle diameter of particulates is 50 nm. A small amount of the liquid dispersion is placed in a Petri dish and the solvent is evaporated to obtain a solid material. The solid material has a number average molecular weight of 11,000,a weight average molecular weight of 18,000, and a glass transition temperature of 65 °C.

### Synthesis of Prepolymer

The following components are placed in a container equipped with a condenser, a stirrer and a nitrogen introducing tube to conduct a reaction at 230 °C at normal pressure for 8 hours followed by another reaction for 5 hours with a reduced pressure of 10 to 15 mmHg to synthesize [Intermediate polyester resin 1]:

| | |
|---|---|
| Adduct of bisphenol A with 2 mole of ethylene oxide | 682 parts |
| Adduct of bisphenol A with 2 mole of propylene oxide | 81 parts |
| Terephthalic acid | 283 parts |
| Trimellitic anhydride | 22 parts |
| Dibutyl tin oxide | 2 parts |

The obtained [Intermediate polyester resin 1] has a number average molecular weight of 2,100, a weight average molecular weight of 9,500, a glass transition temperature of 55 °C, an acid value of 0.5 mgKOH/g and a hydroxyl value of 49 mgKOH/g.

Next, 411 parts of [Intermediate polyester 1], 89 parts of isophorone diisocyanate and 500 parts of ethyl acetate are placed in a reaction container equipped with a condenser, stirrer and a nitrogen introducing tube to conduct reaction at 100 °C for 5 hours to obtain [Prepolymer 1]. The weight % of isolated isocyanate of the obtained [Prepolymer 1] is 1.53 %.

### Synthesis of Master Batch

40 parts of C.I. Solvent Red, 60 parts of binder resin (polyester resin) (RS-801, manufactured by Sanyo Chemical Industries, Ltd., acid value: 10, Mw: 20,000, Tg: 64 °C) and 30 parts of water are mixed by a HENSCHEL MIXER to obtain a mixture in which water sops in a pigment agglomeration body. The mixture is mixed and kneaded for 45 minutes by two rolls where the temperature of the surface is set at 130 °C and pulverized by a pulverizer to the size of 1 mm Φ. Thus, [Master batch 1] is obtained.

### Example 1

### Preparation of Pigment, Wax and Infrared Absorbing Agent Liquid Dispersion (Oil Phase)

543.5 parts of [Polyester 1], 181 parts of paraffin wax (melting point: 72 °C), 6 parts of [Infrared absorbing agent B], 6 parts of [Infrared absorbing agent C] and 1, 450 pars of ethyl acetate are placed in a reaction container equipped with a stirrer and a thermometer. After the system is heated to 80°C while stirring, the system is maintained at 80 °C for 5 hours and then cooled down to 30 °C in one hour. Next, 500 parts of [Master batch 1] and 100 parts of ethyl acetate are placed in the reaction container followed by mixing for about one hour to obtain a [Raw material solution 1].

1,500 parts of [Raw material solution 1] is transferred to a vessel to disperse a pigment, the wax and the infrared absorbing agent using a bead mill (ULTRAVISCOMILL from AIMEX) under the following conditions:
Liquid feeding speed: 1 kg/hour
Disc rotation perimeter speed: 6 m/sec
Diameter of zirconia beads: 0.5 mm
Filling factor of zirconia beads: 80 % by volume
Repeat number of dispersion treatment: 3 times

Next, 655 parts of 65 % ethyl acetate solution of [Polyester 1] is added to the liquid dispersion. After 1 pass of the bead mill under the condition mentioned above, [Pigment, wax and infrared absorbing agent liquid dispersion 1] is obtained. Ethyl acetate added to [Pigment, wax and infrared absorbing agent liquid dispersion 1] to adjust the solid portion density thereof to be 50 % (130 °C, 30 minutes).

### Preparation of Aqueous Phase

968 parts of deionized water, 40 parts of 25 % by weight aqueous liquid dispersion of organic resin particulates (a copolymer of styrene - methacrylic acid - butyl acrylate - a sodium salt of sulfate of an adduct of methacrylic acid with ethyleneoxide) for stabilizing dispersion, 150 parts of 48.5 % aqueous solution of sodium dodecyldiphenyl etherdisulfonate (EREMINOR MON-7, manufactured by Sanyo Chemical Industries, Ltd.), and 98 parts of ethyl acetate are mixed and stirred. Thus, a milk white liquid of [Aqueous phase 1] is obtained.

### Emulsification

976 parts of [Pigment, wax and infrared absorbing agent liquid dispersion 1] and 2.6 parts of isophorone dimaine as an amine are mixed by a TK HOMOMIXER (manufactured by Tokushu Kika Kogyo Co., Ltd.) at a rotation number of 5,000 rpm for one minute. Thereafter, 88 parts of [Prepolymer 1] is admixed by the TK HOMOMIXER (manufactured by Tokushu Kika Kogyo Co., Ltd.) at a rotation number of 5,000 rpm for one minute. Then, 1,200 parts of [Aqueous phase 1] is added and the resultant is mixed by the TK HOMOMIXER (manufactured by Tokushu Kika Kogyo Co., Ltd.) for 20 minutes while controlling the rotation speed thereof in the range of from 8, 000 to 13, 000 rpm to obtain [Emulsified slurry 1].

### Removal of Solvent

[Emulsified slurry 1] is placed in a container equipped with a stirrer and a thermometer and the solvent is removed at 30 °C for 8 hours to obtain [Slurry dispersion 1].

### Particulate Attachment Process

Liquid dispersion of [Vinyl based copolymer resin particulate S-1] is added to [Slurry dispersion 1] with a ratio of 1 to 0.15 with regard to the solid portion and heated to 73 °C in 30 minutes time. A liquid in which 100 parts of hexahydrate of magnesium chlorinate is dissolved in 100 parts of deionized water is added to the resultant little by little while keeping the temperature at 73 °C. After 4 hours, an aqueous solution of hydrochloric acid is added to the resultant to adjust pH thereof to be 5 followed by heating to 80 °C. Subsequent to 2 hour cooling down, [Slurry dispersion 1-2] is obtained.

### Washing and Drying

After 100 parts of [Slurry dispersion 1-2] is filtered with a reduced pressure;
(I) : 100 parts of deionized water is added to the filtered cake and the mixture is mixed by a TK HOMOMIXER at a rotation number of 12,000 rpm for 10 minutes;
(II) : 900 parts of deionized water is added to the filtered cake of (I) and the resultant is mixed by a TK HOMOMIXER at a rotation number of 12, 000 rpm for 30 minutes while applying ultrasonic vibration thereto, and then filtered under a reduced pressure. This operation is repeated until the electric conductivity of the re-slurry liquid is not greater than 10 µC/cm;
(III) : 10 % hydrochloric acid is added to the re-slurry liquid of (II) to make pH thereof to be 4 followed by 30 minute stirring by a three one motor; and
(IV) : 100 parts of deionized water is added to the filtered cake of (III) and the resultant is mixed by a TK HOMOMIXER at a rotation number of 12,000 rpm for 10 minutes followed by filtration. This operation is repeated until the electric conductivity of the re-slurry liquid is not greater than 10 µC/cm. Thus, [Filtered cake 1] is obtained.

[Filtered cake 1] is dried by a circulating drier at 45 °C for 48 hours. The dried cake is sieved using a screen having an opening of 75 µm to obtain [Colored particle 1].

The obtained [Colored particle 1] is subject to external additive treatment as follows:
1.5 parts of hydrophobic silica (BET 200 m²/g) is admixed to 100 parts of [Colored particle 1] by HENSHCEL MIXER FM20C/I (manufactured by Mitsui Mining Co., Ltd.) for 5 minutes to obtain a toner (development agent).

With regard to HENSHCEL MIXER, a combination of upper wing AO and lower wing ST is used with a front speed of the lower wing is fixed at 40 m/s.

### Manufacturing of Fixing Helping Particle

1,698 parts of an adduct of bisphenol A with ethylene oxide (average addition mole number: 2.2) and 163 parts of cyclohexane dimethanol are set in a flask equipped with a stirrer, a nitrogen introducing mouth, a thermometer and a rectification column and heated to 140 °C. Thereafter, 1.4 parts of dibutyltin oxide is placed in the system. After it is confirmed that the system can be uniformly stirred, 943 parts of terephthalic acid and 111 parts of isophthalic acid are gradually placed in the system.

Next, while keeping stirring, the temperature of the system is increased to 220 °C in three hours and to 245 °C in another three hours followed by reaction for 8 hours at the same temperature. As a result, [ Polyester resin P1] having an acid value of 16.0, a softening point of 115 °C according to a ring and ball method, a Tg of 65 °C according to DSC, a number average molecular weight (Mn) of 4,200 and a weight average molecular weight (Mw) of 18,000 according to GPC method.

A liquid dispersion in which 3 parts of the ultrafine particulate D is dispersed in 100 parts of tetrahydrofuran and 100 parts of coarsely-pulverized Polyester resin P1 are set in a glass autoclave having a propeller wing and a pressure of 0.2 MPa is preliminarily applied to the system with nitrogen gas followed by heating the system to 90 °C while rotating the propeller wing at 100 rpm.

The pressure in the autoclave at the time increases to 0.45 Mpa.

When the system is heated to 90 °C, the rotation number of the propeller wing is increased to 900 rpm for stirring for 10 minutes to obtain a resin solution. Thereafter, 400 parts of an aqueous medium preliminarily heated to 90 °C formed of 2.9 parts of 25 % ammonium water and 397.1 parts of deionized water is infused into the system in 5 minutes with an increased pressure to obtain an initial aqueous dispersion body in which a polyester resin is dispersed in water in particulate manner.

The obtained initial aqueous dispersion body is cooled down to 30 °C by water while keeping stirring and then drawn out. Tetrahydrofuran is distilled away under the condition of 47 °C for 30 minutes using a rotary evaporator to obtain a polyester resin particulate aqueous dispersion body. This polyester resin particulate aqueous dispersion body is dried to obtain [Fixing helping particle 1].

The physical properties of obtained Toner 1, the composition of the infrared absorption agent, and the physical properties of [Colored helping particle 1] are shown in Tablea 1-1 and 1-2.

The obtained toner and the colored helping particle are evaluated for each item below. The results are shown in Talbe 2.

### Fixing Property Evaluation

A monochrome non-fixed image is formed by using ipsio CX2500 (manufactured by Ricoh Co. Ltd.). The amount of toner attachment on the sheet is 2 g/m². The fixing helping particle is placed on a mesh and the mesh is vibrated over the non-fixed image so that the fixing helping agent is evenly sprinkled on the non-fixed image. This non-fixed image on which the fixing helping agent is placed is fixed by a flash fixing device (non-contact fixing device) using a Xenon lamp having an oscillation wavelength range having emission spectrum peaks at least in a range of from 810 to 840 nm and a range of from 900 to 980 nm as a light source. The fixing power is 3.0 J/cm² and the transfer speed is 120 mm/sec.

The fixing property is evaluated by the variance in the image density between before and after the fixed image is rubbed by a sand eraser. Ths fixing property index is represented by: (image density after the image is rubbed by a sand eraser / image density therebefore) × 100 (%). The image density is measured by a spectrodensitometer (manufactured by X-Rite Corporation) for evaluation.
G (Good): Variance in image density is 80 % or higher
F (Fair): Cuaing no practical problem (variance in image density is 70 % or higher)
B (Bad) : Cuasing practical problem (variance in image density is less than 70 %)

### Anti-smear Property

The degree of contamination of unused paper when the unused paper is rubbed with the image obtained for the fixing property evaluation is observed and evaluated.
E (Excellent): No contamination observed
G (Good): contamination hardly observed
F (Fair): Contamination observed while causing no practical problem
B (Bad) : Significant contamination observed, which causes a practical problem

### Gloss

Gloss of the image obtained in the fixing property evaluation is compared with a case in which only a non-fixed image is fixed for observation and evaluation. In addition, uneven gloss is observed and evaluated.
E (Excellent) : Gloss is significantly improved with no uneven gloss G (Good) : Gloss is significantly improved with uneven gloss causing no practical problem
F (Fair): Gloss is improved with uneven gloss causing no practical problem
B (Bad): Gloss is not significantly improved or improved but with significant uneven gloss.

### Color Reproducibility

Fixed images of single color toner are obtained in the same manner as in the fixing property evaluation except that the attachment amount of toner is changed to 5 g/m².
G (Good): Good color reproduciibility
F (Fair) : Cloud slightly observed in color without causing a practical problem
B (Bad): Cloud significantly observed in color, which causes a practical problem

### Example 2

In Example 2, the same toner as in Example 1 is used but the fixing helping particle 1 is changed to the following fixing helping particle 2. Example 2 is evaluated in the same manner as in Example 1.

### Manufacturing of Fixing Helping Particle 2

324 parts of ethylene glycol, 545 parts of neopentyl glycol, and 112 parts of trimethylol propane are set in a flask equipped with a stirrer, a nitrogen introducing mouth, a thermometer and a rectification column and heated to 140 °C. Thereafter, 2.4 parts of dibutyltin oxide is placed in the system. After it is confirmed that the system can be uniformly stirred, 1, 808 parts of terephthalic acid is gradually placed in the system.

Next, while keeping stirring, the temperature of the system is increased to 195 °C in three hours and to 240 °C in ten hours followed by reaction for 5 hours at the same temperature. As a result, [Polyester resin P2] is obtained which has a softening point of 113 °C according to a ring and ball method, a Tg of 58 °C according to DSC, a number average particle diameter (Mn) of 3,500 and a weight average molecular weight (Mw) of 20,000 according to GPC method.

A liquid dispersion in which 3 parts of the ultrafine particulate D is dispersed in 100 parts of acetone and 100 parts of coarsely-pulverized Polyester resin P2 are set in a glass autoclave having a propeller wing and a pressure of 0.2 MPa is preliminarily applied to the system with nitrogen gas followed by heating the system to 90 °C while rotating the propeller wing at 100 rpm.

The pressure in the autoclave at the time increases to 0.45 Mpa.

When the system is heated to 90 °C, the rotation number of the propeller wing is increased to 900 rpm for stirring for 10 minutes to obtain a paste swollen body by causing the coarsely-pulverized Polyester resin P2 to absorb acetone.

Thereafter, 400 parts of an aqueous medium preliminarily heated to 90 °C formed of 2.9 parts of 25 % ammonium water and 397.1 parts of deionized water is infused into the system with an increased pressure in 5 minutes to obtain an initial aqueous dispersion body in which the swollen body is dispersed in water in particulate manner.

The obtained initial aqueous dispersion body is cooled down to 30 °C by water while keeping stirring and then drawn out. Acetone is distilled away using a rotary evaporator under the condition of 47 °C for 30 minutes to obtain a polyester resin particulate aqueous dispersion body. This polyester resin particulate aqueous dispersion body is dried to obtain [Fixing helping particle 2].

### Example 3

In Example 3, the same toner as in Example 1 is used but the fixing helping particle 1 is changed to the following fixing helping particle 3. Example 3 is evaluated in the same manner as in Example 1.

### Manufacturing of Fixing Helping Particle 2

324 parts of ethylene glycol, 545 parts of neopentyl glycol, and 112 parts of trimethylol propane are set in a flask equipped with a stirrer, a nitrogen introducing mouth, a thermometer and a rectification column and heated to 140 °C. Thereafter, 2.4 parts of dibutyltin oxide is placed in the system. After it is confirmed that the system can be uniformly stirred, 1, 808 parts of terephthalic acid is gradually placed in the system.

Next, while keeping stirring, the temperature of the system is increased to 195 °C in three hours and to 240 °C in ten hours followed by reaction for 3 hours at the same temperature. As a result, [Polyester resin P3] is obtained which has a softening point of 105 °C according to a ring and ball method, a Tg of 58 °C according to DSC, a number average particle diameter (Mn) of 3,000 and a weight average molecular weight (Mw) of 13,000 according to GPC method.

A liquid dispersion in which 3 parts of the ultrafine particulate D is dispersed in 100 parts of acetone and 100 parts of coarsely-pulverized Polyester resin P3 are set in a glass autoclave having a propeller wing and a pressure of 0.2 MPa is preliminarily applied to the system with nitrogen gas followed by heating the system to 90 °C while rotating the propeller wing at 100 rpm.

When the system is heated to 90 °C, the rotation number of the propeller wing is increased to 900 rpm for stirring for 10 minutes to obtain a translucent paste swollen body by causing the coarsely-pulverized Polyester resin P3 to absorb acetone.

Thereafter, 400 parts of an aqueous medium preliminarily heated to 90 °C formed of 2.9 parts of 25 % ammonium water and 397.1 parts of deionized water is infused into the system in 5 minutes with an increased pressure to obtain an initial aqueous dispersion body in which the swollen body is dispersed in water in particulate manner.

The obtained initial aqueous dispersion body is cooled down to 30 °C by water while keeping stirring and then drawn out. Acetone is distilled away using a rotary evaporator under the condition of 47 °C for 30 minutes to obtain a polyester resin particulate aqueous dispersion body. This polyester resin particulate aqueous dispersion body is dried to obtain [Fixing helping particle 3].

### Example 4

In Example 4, the same toner as in Example 1 is used but the fixing helping particle 1 is changed to the following fixing helping particle 4. Example 4 is evaluated in the same manner as in Example 1.

### Manufacturing of Fixing Helping Particle 4

400 parts of demineralized water is set in a glass reaction container equipped with a stirrer, heating-cooling equipment, a concentrating device, and devices for respective material and helping agents and the system is heated to 90 °C with a nitrogen atmosphere. Thereafter, the following monomer liquid dispersion and emulsification agent aqueous medium are added and dispersed. Then, an initiator is added to the system to conduct emulsification polymerization reaction for 9 hours.

### Monomer Liquid Dispersion

| | |
|---|---|
| Styrene | 79 parts |
| Butyl acrylate | 21 parts |
| Acylic acid | 3 parts |
| Octane thiol | 0.38 parts |
| Hexane diol diacrylate (HDDA) | 0.7 parts |
| Ultrafine particulate D | 3 parts |

### Emulsification Agent Aqueous Solution

| | |
|---|---|
| 10 % dodecyl benzene sodium sulphnate (S-DBS) aqueous solution | 0.7 parts |
| Demineralized water | 25 parts |

### Initiator

| | |
|---|---|
| 8 % hydrogen peroxide solution | 10.6 parts |
| 8 % ascorbic acid solution | 10.6 parts |

Subsequent to the polymerization reaction, the system is cooled down to obtain a polymer liquid dispersion. The obtained polymer liquid dispersion has a weight average molecular weight of 96, 000 and a glass transition temperature (Tg) of 57 °C.

### Example 5

The development agent of Examples 5 is manufactured in the same manner as in Example 1 except that the toner has a volume average volume particle diameter of 4.2 µm.

The fixing helping particle 2 of Example 2 is used and Example 5 is evaluated in the same manner as in Example 1.

### Example 6

The development agent of Example 6 is manufactured in the same manner as in Example 1 except that the content of the infrared absorption agent B is changed from 3 parts to 0 parts and the content of the infrared absorption agent C is changed from 3 parts to 6 parts in Preparation of Pigment, Wax and Infrared Absorbing Agent Liquid Dispersion (Oil Phase).

The fixing helping particle 1 of Example 1 is used and Example 6 is evaluated in the same manner as in Example 1.

### Example 7

In Example 7, the same toner and fixing helping particle as in Example 1 are used.

Example 7 is evaluated in the same manner as in Example 1 except that the amount of toner attachment is changed to 5 g/m² and the toner is fixed with flash. The flash fixing device uses a Xenon lamp having an oscillation wavelength range having emission spectrum peaks at least in a range of from 810 to 840 nm and a range of from 900 to 980 nm as a liaght source and the fixing power is 3.0 J/cm².

### Example 8

The same toner as in Example 1 is used in Example 8.

The fixing helping particle 8, which is classified so as to have a narrow particle size distribution as in Tables 1-1 and 1-2, is used and Example 8 is evaluated in the same manner as in Example 1.

### Comparative Example 1

The same toner as in Example 1 is used in Comparative Example 1 and the fixing helping particle used is the following fixing helping particle H1 and Comparative Example 1 is evaluated in the same manner as in Example 1.

### Manufacturing of Fixing Helping Particle H1

The fixing helping particle H1 is obtained in the same manner as in Example 1 except that the pigment is not added to the toner of Example 1.

### Comparative Example 2

The same toner as in Example 1 is used in Comparative Example 2.

The fixing helping particle H2 is obtained in the same manner as in Example 1 except that the particle size distribution of the fixing helping particle is changed as in Tables 1-1 and 1-2. Comprative Example 2 is evaluated in the same manner as in Example 1.

### Comparative Example 3

The same toner as in Example 1 is used in Comparative Example 3. The fixing helping particle H3 is obtained in the same manner as in Example 1 except that the particle diameter and the circularity of the fixing helping particle are changed as shown in Tables 1-1 and 1-2. Comparative Example 3 is evaluated in the same manner as in Example 1.

### Comparative Example 4

The same toner as in Example 1 is used in Comparative Example 4 and the fixing helping particle H1 is used.

Comparative Example 4 is evaluated in the same manner as in Example 1 except that amount of toner attachment is changed to 5 g/m² and the toner is fixed with flash.

### Comparative Example 5

450 parts of 0.1M-Na₃PO₄ aqueous solution is set in 700 parts of deionized water and the system is heated to 60 °C followed by stirring at 4,500 rpm using Clearmix CLS-30S (manufactured by M Technique Co., Ltd.). 68 parts of 0.1M-CaCl₂ solution is gradually added to the system to obtain an aqueous medium containing calcium phosphate.

The following recipe is heated to 60 °C and uniformly dissolved and dispersed.

| | |
|---|---|
| Styrerne | 160 parts |
| n-butylacrylate | 40 parts |
| C.I. Pigment blue 15:3 | 10 parts |
| di-t-butylsalicylate metal compound | 2 parts |
| Saturated polyester (acid value: 15, peak molecular weight: 12,000) | 10 parts |
| Ester-based wax (melting point: 60 °C) | 30 parts |
| Infrared absorption agent B | 0.25 parts |
| Infrared absorption agent C | 0.25 parts |
| Divinyl benzene | 0.3 parts |

5 parts of 2,2'-azobis(2,4-dimethylvaleronitrile) is dissolved in the liquid as a polymerization initiator to prepare a polymerizable monomer composition.

The polymerizable monomer composition is placed in the aqueous medium and the system is stirred at 65 °C in nitrogen atmosphere using Clearmix at 4, 500 rpm for 15 minutes to granulate polymerizable monomer composition. Thereafter, the polymerizable monomer is heated to 70 °C while being stirred by a paddle stirrer to conduct reaction for 12 hours. Subsequent to the polymerization reaction, the remaining monomer is distilled away at 80 °C under a reduced pressure. After the system is cooled down, hydrochloric acid is added to dissolve calcium phosphate followed by filtration, washing and drying to obtain colored particles.

The colored particles have a weight average molecular weight (Mw) of 500,000.

The colored particle is subject to the same external additive treatment as in Example 1 and the fixing helping particle H2 is used. Comparative Example 5 is evaluated in the same manner as in Example 1.

**Table 1-1**

| Physical Property | | | | | |
|---|---|---|---|---|---|
| | Physical property of colored particle | | | | |
| | Particle diameter | | | Circularity | Tm (softening point) |
| | Dvc (µm) | Dpc (µm) | Dvc/Dpc | Sc | °C |
| Example 1 | 5.7 | 5.0 | 1.14 | 0.97 | 129 |
| Example 2 | 5.7 | 5.0 | 1.14 | 0.97 | 129 |
| Example 3 | 5.7 | 5.0 | 1.14 | 0.97 | 129 |
| Example 4 | 5.7 | 5.0 | 1.14 | 0.97 | 129 |
| Example 5 | 4.2 | 3.6 | 1.17 | 0.97 | 129 |
| Example 6 | 5.7 | 5.0 | 1.14 | 0.97 | 129 |
| Example 7 | 5.7 | 5.0 | 1.14 | 0.97 | 129 |
| Example 8 | 5.7 | 5.0 | 1.14 | 0.97 | 129 |
| Comparative Example 1 | 5.7 | 5.0 | 1.14 | 0.97 | 129 |
| Comparative Example 2 | 5.7 | 5.0 | 1.14 | 0.97 | 129 |
| Comparative Example 3 | 5.7 | 5.0 | 1.14 | 0.97 | 129 |
| Comparative Example 4 | 5.7 | 5.0 | 1.14 | 0.97 | 129 |
| Comparative Example 5 | 7.5 | 6.4 | 1.17 | 0.97 | 130 |

**Table 1-2**

| | Composition of colored particle | | Physical property of fixing helping particle | | | |
|---|---|---|---|---|---|---|
| | Infrared absorption agent B | Infrared absorption agent B | Particle diameter | | | Circulartiy |
| | Weight % | Weight % | Dvt (µm) | Dpt (µm) | Dvt/Dpt | St |
| Example 1 | 0.1 | 0.1 | 510 | 360 | 1.42 | 0.98 |
| Example 2 | 0.1 | 0.1 | 260 | 180 | 1.44 | 0.98 |
| Example 3 | 0.1 | 0.1 | 490 | 340 | 1.44 | 0.98 |
| Example 4 | 0.1 | 0.1 | 450 | 310 | 1.45 | 0.98 |
| Example 5 | 0.1 | 0.1 | 260 | 180 | 1.44 | 0.98 |
| Example 6 | - | 0.2 | 510 | 360 | 1.42 | 0.98 |
| Example 7 | 0.1 | 0.1 | 510 | 360 | 1.42 | 0.98 |
| Example 8 | 0.1 | 0.1 | 460 | 390 | 1.18 | 0.98 |
| Comparative Example 1 | 0.1 | 0.1 | 5700 | 5100 | 1.12 | 0.97 |
| Comparative Example 2 | 0.1 | 0.1 | 1200 | 1050 | 1.14 | 0.98 |
| Comparative Example 3 | 0.1 | 0.1 | 550 | 520 | 1.06 | 0.91 |
| Comparative Example 4 | 0.1 | 0.1 | 5700 | 5100 | 1.12 | 0.97 |
| Comparative Example 5 | 0.1 | 0.1 | 1200 | 1050 | 1.14 | 0.98 |

**Table 2**

| Evaluation Result | | | | |
|---|---|---|---|---|
| | Evaluation result | | | |
| | Fixing property | Anti-smear property | Gloss | Color reproducibility |
| Example 1 | G | G | G | G |
| Example 2 | G | E | E | G |
| Example 3 | G | G | G | G |
| Example 4 | G | G | G | G |
| Example 5 | G | E | E | G |
| Example 6 | G | G | G | G |
| Example 7 | G | G | G | G |
| Example 8 | G | F | G | G |
| Comparative Example 1 | B | B | F | G |
| Comparative Example 2 | B | B | F | G |
| Comparative Example 3 | F | B | B | G |
| Comparative Example 4 | B | F | B | G |
| Comparative Example 5 | B | B | B | G |

## Claims

1. An image formation method comprising:
developing a latent image on an image bearing member with a toner comprising a coloring agent and a first binder resin;
transferring the toner to a recording medium;
transferring a fixing helping particle comprising a second binder resin to the recording medium; and
fixing the toner and the fixing helping particle on the recording medium,
wherein the toner and the fixing helping particle satisfy the following relationships: $6 μm \geq Dvc \geq 3 μm$ $Dvc > 10 \times Dvt$ $Sc < St$
wherein Dvc represents a volume average particle diameter of the toner, Dvt represents a volume average particle diameter of the fixing helping particle, Sc represents an average circularity of the toner and St represents an average circularity of the fixing helping particle.

2. An image formation method according to Claim 1, wherein a non-contact fixing device is used in the step of fixing.

3. The image formation method according to Claim 2, wherein the toner further comprises a first infrared absorption agent and the fixing helping agent further comprises a second infrared absorption agent.

4. The image formation method according to Claim 3, wherein the first infrared absorption agent has a maximum absorption wavelength in a wavelength range of from 700 to 1,100 nm.

5. The image formation method according to Claim 3 or 4, wherein a content of the first infrared absorption agent is from 0.1 to 2 % by weight based on a content of the toner.

6. The image formation method according to any one of Claims 3 to 5, wherein the first infrared absorption agent comprises at least two compounds each having a different maximum absorption wavelength.

7. The image formation method according to any one of Claims 3 to 6, wherein a flash fixing device is used in the step of fixing.

8. The image formation method according to any one of Claims 1 to 7, wherein the fixing helping particle satisfies the following relationship: $Dvt / Dpt > 1.4 ,$
Where Dpt represents a number average particle diameter of the fixing helping particle.

9. The image formation method according to any one of Claims 1 to 8, wherein the first binder resin comprises a polyester based resin.

10. The image formation method according to any one of Claims 1 to 9, wherein the toner has an average circularity not less than 0.95.

11. The image formation method according to any one of Claims 1 to 10, wherein a single component development device is used in the step of developing.

## Patentansprüche

1. Bilderzeugungsverfahren, umfassend:
Entwickeln eines latenten Bildes auf einem Bildträgerelement mit einem Toner, der ein farbgebendes Mittel und ein erstes Bindemittelharz umfasst;
Übertragen des Toners auf ein Aufzeichnungsmedium;
Übertragen eines Fixierhilfsteilchens umfassend ein zweites Bindemittelharz auf das Aufzeichnungsmedium; und
Fixieren des Toners und des Fixierhilfsteilchens auf dem Aufzeichnungsmedium,
wobei der Toner und das Fixierhilfsteilchen die folgenden Beziehungen erfüllen: $6 μm \geq Dvc \geq 3 μm$ $Dvc > 10 x Dvt$ $Sc < St$
wobei Dvc ein Volumenmittel des Teilchendurchmessers des Toners ist, Dvt ein Volumenmittel des Teilchendurchmessers des Fixierhilfsteilchens ist, Sc eine mittlere Zirkularität des Toners ist und St eine mittlere Zirkularität des Fixierhilfsteilchens ist.

2. Bilderzeugungsverfahren nach Anspruch 1, wobei eine berührungsfreie Fixiervorrichtung in dem Schritt der Fixierung verwendet wird.

3. Bilderzeugungsverfahren nach Anspruch 2, wobei der Toner ferner ein erstes Infrarot-Absorptionsmittel umfasst und das Fixierhilfsmittel ferner ein zweites Infrarot-Absorptionsmittel umfasst.

4. Bilderzeugungsverfahren nach Anspruch 3, wobei das erste Infrarot-Absorptionsmittel eine maximale Absorptionswellenlänge in einem Wellenlängenbereich von 700 bis 1.100 nm aufweist.

5. Bilderzeugungsverfahren nach Anspruch 3 oder 4, wobei der Gehalt des ersten Infrarot-Absorptionsmittels von 0,1 bis 2 Gew.-%, bezogen auf den Gehalt des Toners, beträgt.

6. Bilderzeugungsverfahren nach irgendeinem der Ansprüche 3 bis 5, wobei das erste Infrarot-Absorptionsmittel wenigstens zwei Verbindungen umfasst, die jeweils eine unterschiedliche maximale Absorptionswellenlänge aufweisen.

7. Bilderzeugungsverfahren nach irgendeinem der Ansprüche 3 bis 6, wobei eine Blitzlichtfixiervorrichtung in dem Schritt der Fixierung verwendet wird.

8. Bilderzeugungsverfahren nach irgendeinem der Ansprüche 1 bis 7, wobei das Fixierhilfsteilchen die folgende Beziehung erfüllt: $Dvt / Dpt > 1 , 4 ,$
wobei Dpt ein Zahlenmittel des Teilchendurchmessers des Fixierhilfsteilchens ist.

9. Bilderzeugungsverfahren nach irgendeinem der Ansprüche 1 bis 8, wobei das erste Bindemittelharz ein Harz auf Polyesterbasis umfasst.

10. Bilderzeugungsverfahren nach irgendeinem der Ansprüche 1 bis 9, wobei der Toner eine mittlere Zirkularität von nicht weniger als 0,95 aufweist.

11. Bilderzeugungsverfahren nach irgendeinem der Ansprüche 1 bis 10, wobei eine Einkomponenten-Entwicklungsvorrichtung in dem Schritt der Entwicklung verwendet wird.

## Revendications

1. Procédé de formation d'image comprenant :
le développement d'une image latente sur un élément de support d'image avec un toner comprenant un agent colorant et un premier liant résineux ;
le transfert du toner sur un support d'enregistrement ;
le transfert d'une particule d'aide au fixage comprenant un deuxième liant résineux sur le support d'enregistrement ; et
le fixage du toner et de la partie d'aide au fixage sur le support d'enregistrement,
dans lequel le toner et la particule d'aide au fixage satisfont aux relations suivantes : $6 μm \geq Dvc \geq 3 μm$ $Dvc > 10 x Dvt$ $Sc < St$
où Dvc représente un diamètre de particule moyen en volume du toner, Dvt représente un diamètre de particule moyen en volume de la particule d'aide au fixage, Sc représente une circularité moyenne du toner et St représente une circularité moyenne de la particule d'aide au fixage.

2. Procédé de formation d'image selon la revendication 1, dans lequel un dispositif de fixage sans contact est utilisé à l'étape de fixage.

3. Procédé de formation d'image selon la revendication 2, dans lequel le toner comprend en outre un premier agent d'absorption des infrarouges et l'agent d'aide au fixage comprend en outre un deuxième agent d'absorption des infrarouges.

4. Procédé de formation d'image selon la revendication 3, dans lequel le premier agent d'absorption des infrarouges a une longueur d'onde d'absorption maximum dans une plage de longueur d'onde de 700 à 1100 nm.

5. Procédé de formation d'image selon la revendication 3 ou 4, dans lequel une teneur en le premier agent d'absorption des infrarouges est de 0,1 à 2 % en poids sur la base d'une teneur en toner.

6. Procédé de formation d'image selon l'une quelconque des revendications 3 à 5, dans lequel le premier agent d'absorption des infrarouges comprend au moins deux composants ayant chacun une longueur d'onde d'absorption maximum différente.

7. Procédé de formation d'image selon l'une quelconque des revendications 3 à 6, dans lequel un dispositif de fixage par flashage est utilisé à l'étape de fixage.

8. Procédé de formation d'image selon l'une quelconque des revendications 1 à 7, dans lequel la particule d'aide au fixage satisfait à la relation suivante : $Dvt / Dpt > 1 , 4 ,$
où Dpt représente un diamètre de particule moyen en nombre de la particule d'aide au fixage.

9. Procédé de formation d'image selon l'une quelconque des revendications 1 à 8, dans lequel le premier liant résineux comprend une résine à base de polyester.

10. Procédé de formation d'image selon l'une quelconque des revendications 1 à 9, dans lequel le toner a une circularité moyenne qui est égale ou supérieure à 0,95.

11. Procédé de formation d'image selon l'une quelconque des revendications 1 à 10, dans lequel un dispositif de développement à composant unique est utilisé à l'étape de développement.
